



US011181844B2

(12) **United States Patent**  
**Nagaoka et al.**

(10) **Patent No.:** **US 11,181,844 B2**  
(b4) **Date of Patent:** **Nov. 23, 2021**

- (54) **TONER AND METHOD OF PRODUCING TONER**
- (71) Applicant: **CANON KABUSHIKI KAISHA, Tokyo (JP)**
- (72) Inventors: **Tomoya Nagaoka, Tokyo (JP); Daisuke Yoshioka, Suntou-gun (JP); Kazuyuki Sato, Yokohama (JP); Yuta Komiya, Suntou-gun (JP); Tomohisa Sano, Mishima (JP); Takashi Matsui, Mishima (JP)**
- (73) Assignee: **CANON KABUSHIKI KAISHA, Tokyo (JP)**
- (\*) Notice: Subject to any disclaimer, the term of this patent is extended or adjusted under 35 U.S.C. 154(b) by 0 days.
- (21) Appl. No.: **16/880,017**
- (22) Filed: **May 21, 2020**
- (65) **Prior Publication Data**  
US 2020/0379363 A1 Dec. 3, 2020
- (30) **Foreign Application Priority Data**  
May 28, 2019 (JP) ..... JP2019-099365
- (51) **Int. Cl.**  
*G03G 9/08* (2006.01)  
*G03G 9/097* (2006.01)  
*G03G 9/087* (2006.01)
- (52) **U.S. Cl.**  
CPC ..... *G03G 9/09725* (2013.01); *G03G 9/0806* (2013.01); *G03G 9/08711* (2013.01); *G03G 9/08755* (2013.01)
- (58) **Field of Classification Search**  
CPC ..... G03G 9/08711; G03G 9/09725  
USPC ..... 430/109.3  
See application file for complete search history.

(56) **References Cited**

U.S. PATENT DOCUMENTS

- 7,123,862 B2 10/2006 Hasegawa et al.  
7,537,877 B2 5/2009 Yoshioka et al.  
7,544,455 B2 6/2009 Yoshioka et al.  
7,582,401 B2 9/2009 Ogawa et al.  
7,678,523 B2 3/2010 Hiroko et al.  
7,678,524 B2 3/2010 Hasegawa et al.  
7,700,254 B2 4/2010 Moribe et al.  
7,740,998 B2 6/2010 Yamazaki et al.  
7,796,926 B2 9/2010 Matsuda et al.  
7,842,446 B2 11/2010 Yanase et al.  
7,855,042 B2 12/2010 Kobori et al.  
7,923,190 B2 4/2011 Magome et al.  
7,935,467 B2 5/2011 Dojo et al.  
8,057,977 B2 11/2011 Moribe et al.  
8,227,162 B2 7/2012 Sano et al.  
8,426,091 B2 4/2013 Magome et al.  
8,426,094 B2 4/2013 Magome et al.  
8,518,620 B2 8/2013 Dojo et al.  
8,614,044 B2 12/2013 Matsui et al.  
8,778,585 B2 7/2014 Matsui et al.  
8,841,054 B2 9/2014 Dojo et al.  
8,883,389 B2 11/2014 Matsui et al.  
9,097,997 B2 8/2015 Nomura et al.  
9,097,998 B2 8/2015 Yamazaki et al.  
9,128,400 B2 9/2015 Takahashi et al.

- 9,152,065 B2 10/2015 Sano et al.  
9,201,323 B2 12/2015 Nishikawa et al.  
9,213,250 B2 12/2015 Nomura et al.  
9,217,943 B2 12/2015 Matsui et al.  
9,235,151 B2 1/2016 Tanaka et al.  
9,239,528 B2 1/2016 Hasegawa et al.  
9,250,548 B2 2/2016 Nomura et al.  
9,261,804 B2 2/2016 Yamazaki et al.  
9,304,422 B2 4/2016 Matsui et al.  
9,341,970 B2 5/2016 Yoshioka et al.  
9,348,246 B2 5/2016 Magome et al.  
9,354,545 B2 5/2016 Matsui et al.  
9,377,708 B2 6/2016 Magome et al.  
9,442,416 B2 9/2016 Magome et al.  
9,442,419 B2 9/2016 Wakabayashi et al.  
9,551,947 B2 1/2017 Hiroko et al.  
9,581,934 B2 2/2017 Ito et al.  
9,606,462 B2 3/2017 Nomura et al.  
9,658,546 B2 5/2017 Tanaka et al.  
9,804,514 B2 10/2017 Suzumura et al.  
9,804,519 B2 10/2017 Suzumura et al.  
9,829,818 B2 11/2017 Yoshioka et al.  
9,841,692 B2 12/2017 Hasegawa et al.  
9,857,707 B2 1/2018 Tsuda et al.  
9,904,195 B2 2/2018 Matsui et al.  
9,927,728 B2 3/2018 Arimura et al.  
9,946,179 B2 4/2018 Arimura et al.  
9,946,181 B2 4/2018 Hasegawa et al.  
9,964,874 B2 5/2018 Suzumura et al.  
9,964,881 B2 5/2018 Ikejiri et al.  
9,971,262 B2 5/2018 Hasegawa et al.  
9,971,263 B2 5/2018 Fukudome et al.  
9,971,264 B2 5/2018 Sano et al.

(Continued)

FOREIGN PATENT DOCUMENTS

- JP 2014-130243 7/2014  
WO 2018/110593 6/2018

OTHER PUBLICATIONS

Fedor, "A Method for Estimating Both the Solubility Parameters and Molar Volumes of Liquids", Polymer Engineering and Science, vol. 14, No. 2 (1974) 147-54.

(Continued)

*Primary Examiner* — Mark A Chapman

(74) *Attorney, Agent, or Firm* — Venable LLP

(57) **ABSTRACT**

A toner including a toner particle that contains a binder resin and inorganic fine particles, wherein the binder resin contains a polymer A that includes a first monomer unit derived from a first polymerizable monomer and a second monomer unit derived from a second polymerizable monomer that is different from the first polymerizable monomer; the first polymerizable monomer is at least one selected from the group consisting of (meth)acrylate esters having an alkyl group having 18 to 36 carbons; the SP value of the first monomer unit and the SP value of the second monomer unit satisfy a specified relationship; each of the inorganic fine particles contains a substrate containing at least one inorganic element selected from metal elements and metalloid elements, and a coating layer; and the coating layer has a specified structure.

17 Claims, No Drawings

(56)

## References Cited

## U.S. PATENT DOCUMENTS

|                 |         |                  |                 |         |                    |
|-----------------|---------|------------------|-----------------|---------|--------------------|
| 10,012,919 B2   | 7/2018  | Matsui et al.    | 2015/0185658 A1 | 7/2015  | Wakabayashi et al. |
| 10,012,923 B2   | 7/2018  | Sano et al.      | 2015/0220013 A1 | 8/2015  | Nishikawa et al.   |
| 10,101,683 B2   | 10/2018 | Nishikawa et al. | 2016/0139522 A1 | 5/2016  | Yoshiba et al.     |
| 10,151,990 B2   | 12/2018 | Suzuki et al.    | 2016/0161874 A1 | 6/2016  | Yamazaki et al.    |
| 10,156,800 B2   | 12/2018 | Tsuda et al.     | 2016/0378003 A1 | 12/2016 | Arimura et al.     |
| 10,197,934 B2   | 2/2019  | Matsui et al.    | 2019/0041762 A1 | 2/2019  | Yoshiba et al.     |
| 10,228,627 B2   | 3/2019  | Nagashima et al. | 2019/0310564 A1 | 10/2019 | Koshima            |
| 10,241,430 B2   | 3/2019  | Kimura et al.    | 2019/0384192 A1 | 12/2019 | Kagawa et al.      |
| 10,289,016 B2   | 5/2019  | Fukudome et al.  | 2019/0384193 A1 | 12/2019 | Hashimoto et al.   |
| 10,295,920 B2   | 5/2019  | Nishikawa et al. | 2019/0384194 A1 | 12/2019 | Yoshiba et al.     |
| 10,295,921 B2   | 5/2019  | Ohmori et al.    | 2019/0384195 A1 | 12/2019 | Saeki et al.       |
| 10,303,075 B2   | 5/2019  | Tanaka et al.    | 2019/0384197 A1 | 12/2019 | Aoki et al.        |
| 10,310,397 B2   | 6/2019  | Sano et al.      | 2019/0384198 A1 | 12/2019 | Matsui et al.      |
| 10,545,420 B2   | 1/2020  | Kinumatsu et al. | 2019/0384200 A1 | 12/2019 | Kamikura et al.    |
| 10,578,990 B2   | 3/2020  | Tsuda et al.     | 2019/0384202 A1 | 12/2019 | Shirayama et al.   |
| 10,656,545 B2   | 5/2020  | Kamae et al.     | 2020/0081361 A1 | 3/2020  | Yoshiba et al.     |
| 10,698,327 B2   | 6/2020  | Nagashima et al. | 2020/0166861 A1 | 5/2020  | Uratani et al.     |
| 10,732,529 B2 * | 8/2020  | Yoshiba .....    | G03G 9/09741    |         |                    |
| 2005/0209364 A1 | 9/2005  | Yamagishi et al. |                 |         |                    |
| 2006/0121379 A1 | 6/2006  | Dojo et al.      |                 |         |                    |
| 2009/0197192 A1 | 8/2009  | Hiroko et al.    |                 |         |                    |
| 2013/0252167 A1 | 9/2013  | Moribe et al.    |                 |         |                    |
| 2014/0004460 A1 | 1/2014  | Yoshiba et al.   |                 |         |                    |

|                 |         |                    |
|-----------------|---------|--------------------|
| 2015/0185658 A1 | 7/2015  | Wakabayashi et al. |
| 2015/0220013 A1 | 8/2015  | Nishikawa et al.   |
| 2016/0139522 A1 | 5/2016  | Yoshiba et al.     |
| 2016/0161874 A1 | 6/2016  | Yamazaki et al.    |
| 2016/0378003 A1 | 12/2016 | Arimura et al.     |
| 2019/0041762 A1 | 2/2019  | Yoshiba et al.     |
| 2019/0310564 A1 | 10/2019 | Koshima            |
| 2019/0384192 A1 | 12/2019 | Kagawa et al.      |
| 2019/0384193 A1 | 12/2019 | Hashimoto et al.   |
| 2019/0384194 A1 | 12/2019 | Yoshiba et al.     |
| 2019/0384195 A1 | 12/2019 | Saeki et al.       |
| 2019/0384197 A1 | 12/2019 | Aoki et al.        |
| 2019/0384198 A1 | 12/2019 | Matsui et al.      |
| 2019/0384200 A1 | 12/2019 | Kamikura et al.    |
| 2019/0384202 A1 | 12/2019 | Shirayama et al.   |
| 2020/0081361 A1 | 3/2020  | Yoshiba et al.     |
| 2020/0166861 A1 | 5/2020  | Uratani et al.     |

## OTHER PUBLICATIONS

U.S. Appl. No. 16/819,736, Kazuyuki Soto, filed Mar. 16, 2020.  
 U.S. Appl. No. 16/868,635, Yuta Komiya, filed May 7, 2020.  
 U.S. Appl. No. 16/907,814, Takashi Matsui, filed Jun. 22, 2020.  
 U.S. Appl. No. 16/910,301, Daisuke Yoshiba, filed Jun. 24, 2020.

\* cited by examiner

## 1

TONER AND METHOD OF PRODUCING  
TONER

## BACKGROUND OF THE INVENTION

## Field of the Invention

The present disclosure relates to a toner used in electro-photographic methods, electrostatic recording methods, and toner jet system recording methods, and to a method of producing the toner.

## Description of the Related Art

There is increasing demand for greater energy conservation and higher speeds from image-forming devices that use electrophotographic methods. In order to respond to this, there is increasing need for the toner to exhibit an excellent low-temperature fixability, i.e., the ability to undergo fixing with small amounts of heat.

Lowering the glass transition point (Tg) of the binder resin in toner is an example of a method for realizing an excellent low-temperature fixability. However, while toner having a reduced Tg can provide a good fixed image at lower temperatures, it has been difficult for this to coexist with the heat-resistant storability.

Methods that use a crystalline resin as the main binder have thus been investigated in order to bring about coexistence between the low-temperature fixability and the heat-resistant storability. When the viscoelasticity of a crystalline resin is measured by gradually raising the temperature from room temperature during a dynamic viscoelastic measurement, the viscosity undergoes very little change up the melting point, while at the melting point plastification suddenly occurs and a sharp drop in the viscosity also occurs accompanying this. As a consequence, crystalline resins exhibit an excellent sharp melt property and have thus received attention as materials that provide coexistence between the low-temperature fixability and heat-resistant storability.

However, the molecular chains in a crystalline resin are oriented with a certain regularity, and as a consequence crystalline resins exhibit the behavior of readily undergoing brittle cracking. Due to this, toner that contains large amounts of a crystalline resin is not robust to external stresses, e.g., stirring in the developing device, and thus exhibits durability problems.

In addition, in an image-forming device that has been sped up, the printed recording paper is discharged via a short paper path and the toner, which has been melted during passage through the fixing nip, is placed under a substantial load prior to satisfactory solidification. The following problems are generated as a consequence: the problem of adhesion of the loaded recording paper and a failure to release; and the problem of the release of the toner that has undergone one fixing process and its transfer to another sheet of paper. These are known as the problems associated with discharged paper adhesion. These phenomena are readily produced with toner that has been provided with low-temperature fixability in order to accommodate high-speed printing.

A variety of proposals have been made to date with regard to improving the low-temperature fixability, heat-resistant storability, durability, or discharged paper adhesion behavior of toner that uses a crystalline resin as the main binder.

Japanese Patent Application Laid-open No. 2014-130243 proposes a toner that uses the following in the binder resin

## 2

of a toner core: a crystalline vinyl resin provided by the copolymerization of a long-chain alkyl group-bearing polymerizable monomer and a polymerizable monomer that forms an amorphous segment.

WO 2018/110593 proposes a toner that uses a binder resin from a long-chain alkyl group-bearing polymerizable monomer and a polymerizable monomer that forms an amorphous segment, wherein the difference between the SP values of the polymerizable monomers is controlled into a certain range.

## SUMMARY OF THE INVENTION

The binder resin used in the toner described in Japanese Patent Application Laid-open No. 2014-130243 exhibits coexistence between the low-temperature fixability and the heat-resistant storability. However, the binder resin used in this toner has a high content of the structure derived from the long-chain alkyl group-bearing polymerizable monomer and exhibits a low elasticity around room temperature, and due to this the durability readily declines. In addition, there is no mention of the discharged paper adhesion behavior and the discussion on controlling the crystalline state is inadequate, and thus there is room for improvement.

On the other hand, the binder resin used in the toner described in WO 2018/110593 exhibits coexistence at a higher level between the low-temperature fixability and the heat-resistant storability. However, there is no discussion of the discharged paper adhesion behavior or the durability, which are problems for toner that uses a crystalline resin as the binder resin, and there is thus room for improvement.

The present disclosure provides a toner that solves the problems identified above. That is, the present disclosure provides a toner that exhibits an excellent low-temperature fixability, heat-resistant storability, durability, and discharged paper adhesion behavior.

The present disclosure is a toner comprising a toner particle that contains a binder resin and inorganic fine particles, wherein

the binder resin contains a polymer A that includes a first monomer unit derived from a first polymerizable monomer, and a second monomer unit derived from a second polymerizable monomer that is different from the first polymerizable monomer;

the first polymerizable monomer is at least one selected from the group consisting of (meth)acrylate esters having an alkyl group having 18 to 36 carbons;

where  $SP_{11}$  ( $J/cm^3$ )<sup>0.5</sup> designates an SP value of the first monomer unit and  $SP_{21}$  ( $J/cm^3$ )<sup>0.5</sup> designates an SP value of the second monomer unit, the following formula (1) is satisfied:

$$3.00 \leq (SP_{21} - SP_{11}) \leq 25.00 \quad (1)$$

each of the inorganic fine particles contains a substrate containing at least one inorganic element selected from metal elements and metalloid elements, and

a coating layer; and

the coating layer has a structure represented by at least one selected from the group consisting of the following formulas (A), (B), (C), and (D).

Moreover, the present disclosure is a toner comprising a toner particle that contains a binder resin and inorganic fine particles, wherein

the binder resin contains a polymer A that is a polymer of a composition containing

a first polymerizable monomer, and a second polymerizable monomer that is different from the first polymerizable monomer;

the first polymerizable monomer is at least one selected from the group consisting of (meth)acrylate esters having an alkyl group having 18 to 36 carbons;

where  $SP_{12}$  ( $J/cm^3$ )<sup>0.5</sup> designates an SP value of the first polymerizable monomer and  $SP_{22}$  ( $J/cm^3$ )<sup>0.5</sup> designates an SP value of the second polymerizable monomer, the following formula (2) is satisfied:

$$0.60 \leq (SP_{22} - SP_{12}) \leq 15.00 \quad (2),$$

each of the inorganic fine particles contains a substrate containing at least one inorganic element selected from metal elements and metalloid elements, and a coating layer; and the coating layer has a structure represented by at least one selected from the group consisting of the following formulas (A), (B), (C), and (D).



Wherein M each independently represents one or more elements selected from the group consisting of tetravalent Si, tetravalent Ti, and tetravalent Zr; M' each independently represents one or more elements selected from the group consisting of trivalent Ti, trivalent Zr, and trivalent Al; each R<sup>1</sup> independently represents an alkyl group or a derivative thereof; R<sup>2</sup> to R<sup>7</sup> each independently represent a hydrogen atom, hydroxy group, —O—\* or a group selected from the group consisting of alkoxy groups, alkyl groups, and derivatives thereof; \* represents a bonding segment to the inorganic element; and n and m each independently represent a positive integer equal to or greater than 1.

Further, the present disclosure is a toner comprising a toner particle that contains a binder resin and inorganic fine particles, wherein

the binder resin contains a polymer A that includes a first monomer unit derived from a first polymerizable monomer, and

a second monomer unit derived from a second polymerizable monomer that is different from the first polymerizable monomer;

the first polymerizable monomer is at least one selected from the group consisting of (meth)acrylate esters having an alkyl group having 18 to 36 carbons;

where  $SP_{11}$  ( $J/cm^3$ )<sup>0.5</sup> designates an SP value of the first monomer unit and  $SP_{21}$  ( $J/cm^3$ )<sup>0.5</sup> designates an SP value of the second monomer unit, the following formula (1) is satisfied:

$$3.00 \leq (SP_{21} - SP_{11}) \leq 25.00 \quad (1);$$

each of the inorganic fine particles contains a substrate containing at least one inorganic element selected from metal elements and metalloid elements; and

the substrate has been treated with a compound that has an alkoxy group and an alkyl group.

Furthermore, the present disclosure is a method of producing the toner according to claim 1, the method comprising:

a step of forming, in an aqueous medium, a particle of a polymerizable monomer composition that contains a polymerizable monomer; and  
25 a step of obtaining the toner particle containing a polymer A obtained by polymerizing the polymerizable monomer contained in the particle.

According to the present disclosure, a toner that exhibits an excellent low-temperature fixability, heat-resistant storability, durability, and discharged paper adhesion behavior can be provided.

Further features of the present invention will become apparent from the following description of exemplary embodiments.

### 35 DESCRIPTION OF THE EMBODIMENTS

Unless specifically indicated otherwise, the expressions “from XX to YY” and “XX to YY” that show numerical value ranges refer in the present disclosure to numerical value ranges that include the lower limit and upper limit that are the end points.

In the present disclosure, “(meth)acrylate ester” means acrylate ester and/or methacrylate ester.

The “monomer unit” in the present disclosure refers to the reacted state of the monomer material in the polymer. For example, one unit is taken to be one carbon-carbon bond segment in a main chain provided by the polymerization of a vinyl monomer into a polymer.

Vinyl monomers can be represented by the following formula (Z):



wherein, Z<sub>1</sub> represents a hydrogen atom or alkyl group (preferably an alkyl group having 1 to 3 carbons and more preferably the methyl group) and Z<sub>2</sub> represents any substituent.

A “crystalline resin” denotes a resin that displays a distinct endothermic peak in measurement by differential scanning calorimetry (DSC).

Crystalline vinyl resins generally have a long-chain alkyl group side chain on the main chain skeleton and exhibit

crystallinity as a resin through crystallization between the long-chain alkyl groups in side chain position.

Thus, when a long-chain alkyl group-bearing crystalline vinyl resin is used, a higher content of the long-chain alkyl group results in an increase in the crystallinity and an increase in the melting point, and, accompanying this, in the appearance of a sharp melt property and an excellent low-temperature fixability and an excellent heat-resistant storability.

However, the elasticity of the crystalline vinyl resin around room temperature declines when the long-chain alkyl group content is high. The toner becomes brittle as a result and a decline in the durability then readily occurs.

On the other hand, the crystallinity undergoes an extreme decline and the melting point is reduced when, in order to ameliorate this decline in the durability, the content of the long-chain alkyl group is brought to or below a certain level by carrying out copolymerization between a long-chain alkyl group-bearing polymerizable monomer and another polymerizable monomer. This results in a decline in the heat-resistant storability, a decline in the sharp melt property, and also a decline in the low-temperature fixability.

Moreover, when toner that has a crystalline portion is temporarily melted during the fixing step, a part of the crystalline portion compatibilizes with the amorphous portion and either its crystallinity is never recovered or some time is required for the crystallinity to be recovered. The following problems of discharged paper adhesion (discharged paper adhesion behavior) readily occur when the discharged paper is loaded in this condition: the problem of separate sheets of paper sticking to one another with a failure of release from one another, and the problem of the release of the fixed toner and its transfer to another sheet of paper. As a consequence, coexistence between the low-temperature fixability and the discharged paper adhesion behavior has been a major problem to date.

As a result of intensive investigations, the present inventors discovered that this problem is solved by controlling the type of the long-chain alkyl group-bearing monomer unit and the other monomer unit and the difference in their SP values and by the co-use of inorganic fine particles having a prescribed coating layer.

The present disclosure is a toner comprising a toner particle that contains a binder resin and inorganic fine particles, wherein

the binder resin contains a polymer A that includes a first monomer unit derived from a first polymerizable monomer, and

a second monomer unit derived from a second polymerizable monomer that is different from the first polymerizable monomer;

the first polymerizable monomer is at least one selected from the group consisting of (meth)acrylate esters having an alkyl group having 18 to 36 carbons;

where  $SP_{11}$  ( $J/cm^3$ )<sup>0.5</sup> designates an SP value of the first monomer unit and  $SP_{21}$  ( $J/cm^3$ )<sup>0.5</sup> designates an SP value of the second monomer unit, the following formula (1) is satisfied:

$$3.00 \leq (SP_{21} - SP_{11}) \leq 25.00 \quad (1)$$

each of the inorganic fine particles contains a substrate containing at least one inorganic element selected from metal elements and metalloid elements, and a coating layer; and

the coating layer has a structure represented by at least one selected from the group consisting of the following formulas (A), (B), (C), and (D).

Moreover, the present disclosure is a toner comprising a toner particle that contains a binder resin and inorganic fine particles, wherein

the binder resin contains a polymer A that is a polymer of a composition containing

a first polymerizable monomer, and

a second polymerizable monomer that is different from the first polymerizable monomer;

the first polymerizable monomer is at least one selected from the group consisting of (meth)acrylate esters having an alkyl group having 18 to 36 carbons;

where  $SP_{12}$  ( $J/cm^3$ )<sup>0.5</sup> designates an SP value of the first polymerizable monomer and  $SP_{22}$  ( $J/cm^3$ )<sup>0.5</sup> designates an SP value of the second polymerizable monomer, the following formula (2) is satisfied:

$$0.60 \leq (SP_{22} - SP_{12}) \leq 15.00 \quad (2)$$

each of the inorganic fine particles contains a substrate containing at least one inorganic element selected from metal elements and metalloid elements, and

a coating layer; and

the coating layer has a structure represented by at least one selected from the group consisting of the following formulas (A), (B), (C), and (D).



Wherein M each independently represents one or more elements selected from the group consisting of tetravalent Si, tetravalent Ti, and tetravalent Zr; M' each independently represents one or more elements selected from the group consisting of trivalent Ti, trivalent Zr, and trivalent Al; each R<sup>1</sup> independently represents an alkyl group or a derivative thereof; R<sup>2</sup> to R<sup>7</sup> each independently represent a hydrogen atom, hydroxy group, —O—\* or a group selected from the group consisting of alkoxy groups, alkyl groups, and derivatives thereof; \* represents a bonding segment to the inor-

ganic element; and n and m each independently represent a positive integer equal to or greater than 1.

Further, the present disclosure is a toner comprising a toner particle that contains a binder resin and inorganic fine particles, wherein

the binder resin contains a polymer A that includes a first monomer unit derived from a first polymerizable monomer, and a second monomer unit derived from a second polymerizable monomer that is different from the first polymerizable monomer;

the first polymerizable monomer is at least one selected from the group consisting of (meth)acrylate esters having an alkyl group having 18 to 36 carbons;

where  $SP_{11}$  ( $J/cm^3$ )<sup>0.5</sup> designates an SP value of the first monomer unit and  $SP_{21}$  ( $J/cm^3$ )<sup>0.5</sup> designates an SP value of the second monomer unit, the following formula (1) is satisfied:

$$3.00 \leq (SP_{21} - SP_{11}) \leq 25.00 \quad (1)$$

each of the inorganic fine particles contains a substrate containing at least one inorganic element selected from metal elements and metalloid elements; and

the substrate has been treated with a compound that has an alkoxy group and an alkyl group.

The SP value referenced here is an abbreviation for solubility parameter and is a value that acts as an index for solubility. The procedure for its calculation is described below.

The polymer A occurs as a resin that exhibits crystallinity because the first polymerizable monomer is at least one selected from the group consisting of (meth)acrylate esters having an alkyl group having 18 to 36 carbons. The melting point of the polymer A can be controlled into a preferred range (for example, from 50° C. to 80° C.) when the number of carbons is in the indicated range.

Where  $SP_{11}$  ( $J/cm^3$ )<sup>0.5</sup> designates the SP value of the first monomer unit and  $SP_{21}$  ( $J/cm^3$ )<sup>0.5</sup> designates the SP value of the second monomer unit, the following formula (1) is satisfied.

Where  $SP_{12}$  ( $J/cm^3$ )<sup>0.5</sup> designates the SP value of the first polymerizable monomer and  $SP_{22}$  ( $J/cm^3$ )<sup>0.5</sup> designates the SP value of the second polymerizable monomer, the following formula (2) is satisfied.

$$3.00 \leq (SP_{21} - SP_{11}) \leq 25.00 \quad (1)$$

$$0.60 \leq (SP_{22} - SP_{12}) \leq 15.00 \quad (2)$$

The value of  $(SP_{21} - SP_{11})$  is preferably 4.00 to 20.00 and is more preferably 5.00 to 15.00.

The value of  $(SP_{22} - SP_{12})$  is preferably 2.00 to 10.00 and is more preferably 3.00 to 7.00.

The unit for the SP value in the present disclosure is  $(J/m^3)^{0.5}$ , but this can be converted to the  $(cal/cm^3)^{0.5}$  unit using the following formula.

$$1 \text{ (cal/cm}^3\text{)}^{0.5} = 2.045 \times 10^3 \text{ (J/m}^3\text{)}^{0.5}$$

By satisfying formula (1) or formula (2), there is no reduction in the crystallinity of the polymer A and its melting point is maintained.

The crystallinity of the polymer A can be controlled at an even higher level by having the toner particle contain, in addition to the polymer A, inorganic fine particles, each of the inorganic fine particles containing a substrate containing a specified inorganic element and a coating layer having a specified structure (that is, the substrate has been treated with a specified compound). Doing this makes it possible for

all of the following to coexist: the low-temperature fixability, the heat-resistant storability, the durability, and the discharged paper adhesion behavior.

The reasons for this are hypothesized as follows.

5 The first monomer unit generates crystallinity through its incorporation in the polymer A and aggregation between/ among the first monomer units. However, when another monomer unit is incorporated, as a general matter this other monomer unit will readily interfere with the crystallization 10 of the first monomer unit, resulting in an impaired generation of crystallinity for the polymer. This trend becomes substantial when the first monomer unit and another monomer unit are randomly bonded in the individual polymer molecule.

15 On the other hand, it is thought that, through the use of polymerizable monomers for which  $(SP_{22} - SP_{12})$  resides in the range given by formula (2), during polymerization the first polymerizable monomer and the second polymerizable monomer do not engage in random polymerization and to a certain degree assume a continuous polymerization mode. Due to the presence of the difference in the SP values when 20  $(SP_{22} - SP_{12})$  is in the range of formula (2), it is thought that polymer segments containing the monomer unit derived from the first polymerizable monomer and polymer segments containing the monomer unit derived from the second polymerizable monomer can form a phase-separated state at a microregional level.

25 It is also thought that, by having  $(SP_{21} - SP_{11})$  be in the range of formula (1), the first monomer unit and the second monomer unit in the polymer A are not compatible and can form a distinct phase-separated state.

30 As a consequence, by having the SP values satisfy formula (1) or (2), it is thought that a polymer segment can then be obtained in which the first polymerizable monomer has undergone continuous polymerization to a certain degree and the crystallinity of the polymer segment can be increased and the melting point is maintained.

35 That is, the polymer A preferably has a crystalline segment containing the first monomer unit derived from the first polymerizable monomer and a high-polarity segment (or amorphous segment) containing the second monomer unit derived from the second polymerizable monomer.

40 A high-polarity segment originating with the M-O bond and a low-polarity segment originating with the alkyl group or derivative thereof are present in the coating layer having a structure represented by at least one selected from the group consisting of formulas (A) to (D).

45 When a polymer A-containing toner particle contains inorganic fine particles having the coating layer as described above, it is thought that the second monomer unit, which is derived from the high-polarity second polymerizable monomer, engages in a dipole-dipole interaction with the high-polarity segment in the coating layer on the inorganic fine particles. It is also thought that an intermolecular force acts 50 between the first monomer unit, which is derived from the low-polarity first polymerizable monomer, and the low-polarity segment in the coating layer on the inorganic fine particles. It is hypothesized that, as a result, the polymer A orients to the inorganic fine particle surface with the first monomer unit as the outside and the second monomer unit as the inside and the crystallinity of the polymer A is further increased and the crystalline state is made uniform.

55 Accordingly, as compared to the absence of the inorganic fine particles, recrystallization post-fixing is faster and the discharged paper adhesion behavior is improved. In addition, due to the higher crystallinity, the sharp melt property is enhanced and the low-temperature fixability and the

heat-resistant storability can coexist at an even higher level. Moreover, because the crystalline state is uniform, stresses applied to the toner, e.g., during stirring in the developer container, are dispersed and the durability is thus enhanced.

When  $(SP_{22}-SP_{12})$  is smaller than  $0.60 (J/cm^3)^{0.5}$ , the melting point of the polymer A declines and the heat-resistant storability declines. In addition, due to the small magnitude taken on by the dipole-dipole interaction between the high-polarity second monomer unit in the polymer A and the high-polarity segment in the coating layer on the inorganic fine particles, the crystallinity becomes small and the discharged paper adhesion behavior declines.

When, on the other hand,  $(SP_{22}-SP_{12})$  is larger than  $15.00 (J/cm^3)^{0.5}$ , the copolymerizability of the polymer A is thought to deteriorate and nonuniformity is generated and the low-temperature fixability declines.

Similarly, when  $(SP_{21}-SP_{11})$  is smaller than  $3.00 (J/cm^3)^{0.5}$ , the melting point of the polymer A declines and the heat-resistant storability declines. In addition, due to the small magnitude taken on by the dipole-dipole interaction between the high-polarity second monomer unit in the polymer A and the high-polarity segment in the coating layer on the inorganic fine particles, the crystallinity becomes small and the discharged paper adhesion behavior declines.

When, on the other hand,  $(SP_{21}-SP_{11})$  is larger than  $25.00 (J/cm^3)^{0.5}$ , the copolymerizability of the polymer A is thought to deteriorate and nonuniformity is generated and the low-temperature fixability declines.

When the inorganic fine particles lack the prescribed coating layer, that is, when the substrate has not been treated with the prescribed compound, the enhancing effect for the crystallinity of the polymer A is poor and nonuniformity of the polymer A is also produced.

That is, the crystallinity of the polymer A can be controlled and the low-temperature fixability, heat-resistant storability, durability, and discharged paper adhesion behavior can be made to coexist by controlling the type and content of the long-chain alkyl group-bearing monomer unit and the other monomer unit and the difference in their SP values and by the co-use of inorganic fine particles having the prescribed coating layer.

When the polymer A contains a plurality of species of monomer units that satisfy the requirements for the aforementioned first monomer unit, the value provided by the weighted-averaging of the SP values of each of these monomer units is used for the value of  $SP_{11}$  in formula (1). For example, the SP value ( $SP_{11}$ ) is expressed by the following formula (6) when a monomer unit A having an SP value of  $SP_{111}$  is contained at A mol % with reference to the number of moles of all the monomer units that satisfy the requirements for the first monomer unit and a monomer unit B having an SP value of  $SP_{112}$  is contained at (100-A) mol % with reference to the number of moles of all the monomer units that satisfy the requirements for the first monomer unit.

$$SP_{11} = (SP_{111} \times A + SP_{112} \times (100-A)) / 100 \quad (6)$$

The calculations are similarly performed when three or more monomer units that satisfy the requirements for the first monomer unit are incorporated.  $SP_{12}$ , on the other hand, also represents the average value similarly calculated using the molar ratios of the respective first polymerizable monomers.

On the other hand, the monomer unit derived from the second polymerizable monomer applies to all monomer units having an  $SP_{21}$  that satisfies formula (1) with respect to  $SP_{11}$  as calculated by the aforementioned method. Similarly, the second polymerizable monomer applies to all

polymerizable monomers having an  $SP_{22}$  that satisfies formula (6) with respect to  $SP_{12}$  as calculated by the aforementioned method.

That is, when the second polymerizable monomer is two or more species of polymerizable monomers,  $SP_{21}$  represents the SP value of the monomer unit derived from each polymerizable monomer and  $SP_{21}-SP_{11}$  is determined for the monomer unit derived from each second polymerizable monomer. Similarly,  $SP_{22}$  represents the SP value of each polymerizable monomer and  $SP_{22}-SP_{12}$  is determined for each second polymerizable monomer.

Each of the inorganic fine particles contains a substrate containing at least one inorganic element selected from metal elements and metalloid elements.

The metal elements can be exemplified by K, Mg, Ca, Sr, Ba, Ti, V, Cr, Mn, Fe, Co, Ni, Cu, Zn, Y, Zr, Nb, Mo, Pd, Ag, Cd, Nd, W, Pt, Au, and Al.

The metalloid elements can be exemplified by Si and Ge.

The substrate containing at least one inorganic element selected from the aforementioned metal elements and metalloid elements can be exemplified by silica, diatomaceous earth, alumina, zinc oxide, titania, zirconia, calcium oxide, calcium carbonate, magnesium oxide, iron oxide, copper oxide, kaolin, clay, talc, mica, glass fibers, potassium titanate, calcium titanate, magnesium titanate, barium titanate, carbon black, and other inorganic materials.

Examples are iron oxides such as magnetite, maghemite, ferrite, and iron oxides that contain another metal oxide, and metals such as Fe, Co, and Ni or alloys of these metals with a metal such as Al, Co, Cu, Pb, Mg, Ni, Sn, Sb, Ca, Mn, Se, and Ti, and mixtures of the preceding. Specific examples are magnetite, iron(III) oxide ( $\gamma\text{-Fe}_2\text{O}_3$ ), zinc iron oxide ( $\text{ZnFe}_2\text{O}_4$ ), copper iron oxide ( $\text{CuFe}_2\text{O}_4$ ), neodymium iron oxide ( $\text{NdFe}_2\text{O}_3$ ), barium iron oxide ( $\text{BaFe}_{12}\text{O}_{19}$ ), magnesium iron oxide ( $\text{MgFe}_2\text{O}_4$ ), and manganese iron oxide ( $\text{MnFe}_2\text{O}_4$ ).

Among the preceding, metal oxides and metalloid oxides are more preferred from the standpoints of the strength of reactivity with the surface treatment agent, the uniformity of treatment, and the practicality for toner applications, with magnetite being even more preferred.

The number-average particle diameter of the inorganic fine particles is preferably  $0.10 \mu\text{m}$  to  $0.40 \mu\text{m}$  and is more preferably  $0.10 \mu\text{m}$  to  $0.25 \mu\text{m}$ . When the number-average particle diameter of the inorganic fine particles is  $0.10 \mu\text{m}$  or more, the uniform dispersibility in the toner is enhanced. When the number-average particle diameter of the inorganic fine particles is  $0.40 \mu\text{m}$  or less, a surface area of the inorganic fine particle is enlarged. Thus, a larger nucleating agent effect can be obtained by having the particle diameter of the inorganic fine particles be in the indicated range.

The content of the inorganic fine particles, per 100 mass parts of the binder resin, is preferably from 20 mass parts to 150 mass parts and is more preferably from 50 mass parts to 100 mass parts. By having the content of the inorganic fine particles be in the indicated range, a toner can be obtained in which the characteristics of both the inorganic fine particles and the binder resin are satisfactorily expressed.

Each of the inorganic fine particles also contains a coating layer. The coating layer has a structure represented by at least one selected from the group consisting of the following formulas (A), (B), (C), and (D):



wherein

M each independently represents one or more elements selected from the group consisting of tetravalent Si, tetravalent Ti, and tetravalent Zr;

M' each independently represents one or more elements selected from the group consisting of trivalent Ti, trivalent Zr, and trivalent Al;

R<sup>1</sup> each independently represents an alkyl group (preferably having 1 to 20 carbons, more preferably having 4 to 16 carbons, and still more preferably having 4 to 10 carbons) or a derivative thereof;

R<sup>2</sup> to R<sup>7</sup> each independently represent a hydrogen atom, hydroxy group, —O—\* or a group selected from the group consisting of alkoxy groups, alkyl groups (preferably having 1 to 20 carbons, more preferably having 4 to 16 carbons, and still more preferably having 4 to 10 carbons), and derivatives thereof; \* represents a bonding segment to the inorganic element; and

n and m each independently represent a positive integer equal to or greater than 1.

The alkyl group derivatives that can be represented by R<sup>1</sup> to R<sup>7</sup> can be specifically exemplified by the butylcyclopentyl group, butylcyclohexyl group, hexylcyclopentyl group, and hexylcyclohexyl group.

The alkoxy group derivatives that can be represented by R<sup>2</sup> to R<sup>7</sup> can be specifically exemplified by the dicyclopentylmethoxy group, dicyclohexylmethoxy group, tricyclopentylmethoxy group, tricyclohexylmethoxy group, phenylmethoxy group, diphenylmethoxy group, and triphenylmethoxy group.

In order to obtain the structures indicated above, preferably the substrate is treated with a compound that has an alkoxy group and an alkyl group (also referred to herebelow as the surface treatment agent). That is, the inorganic fine particles are preferably the reaction product of a substrate and the surface treatment agent.

Specifically, the substrate is preferably treated with a compound such as, e.g., a silane compound, titanate compound, aluminate compound, zirconate compound, and so

forth. That is, the inorganic fine particles are preferably the reaction product of the substrate and a compound such as, e.g., a silane compound, titanate compound, aluminate compound, zirconate compound, and so forth.

- 5 All of these surface treatment agents form strong chemical bonds by undergoing hydrolysis and a condensation reaction with the hydroxyl groups present on the surface of the inorganic fine particles. Due—in the case of a toner that contains the inorganic fine particles and the polymer A—to  
10 the presence of a structure as described above in the coating layer of the inorganic fine particles, dipole-dipole interactions occur between the second monomer unit, which is derived from the high-polarity second polymerizable monomer, and the high-polarity segment in the coating layer on the inorganic fine particles. In addition, an intermolecular force acts between the first monomer unit, which is derived from the low-polarity first polymerizable monomer, and the low-polarity segment in the coating layer on the inorganic fine particles. As a result, the polymer A orients to the  
15 inorganic fine particle surface with the first monomer unit as the outside and the second monomer unit as the inside, and the crystallinity of the polymer A is further increased and the crystalline state is made uniform.

The silane compound can be exemplified by methyltrimethoxysilane, ethyltrimethoxysilane, dimethyltrimethoxysilane, methyltriethoxysilane, dimethyltriethoxysilane, n-butyltrimethoxysilane, n-dibutyltrimethoxysilane, n-butyltriethoxysilane, n-dibutyltriethoxysilane, isobutyltrimethoxysilane, trimethylmethoxysilane, n-hexyltrimethoxysilane, n-octyltrimethoxysilane, n-octyltriethoxysilane, n-decyldimethoxysilane, n-decyltrimethoxysilane, n-decyltriethoxysilane, n-didecyldimethoxysilane, n-decyltriethoxysilane, n-didecyltriethoxysilane, n-hexadecyltrimethoxysilane, n-hexadecyltriethoxysilane, and n-octadecyltrimethoxysilane, and hydroxylates of the preceding.

The titanate compound can be exemplified by methyltrimethoxytitanium, dimethyltrimethoxytitanium, methyltriethoxytitanium, dimethyltriethoxytitanium, n-butyltrimethoxytitanium, n-dibutyltrimethoxytitanium, n-butyltriethoxytitanium, n-dibutyltriethoxytitanium, isobutyltrimethoxytitanium, trimethylmethoxytitanium, n-hexyltrimethoxytitanium, n-octyltrimethoxytitanium, n-octyltriethoxytitanium, n-decyltrimethoxytitanium, n-decyltriethoxytitanium, n-didecyldimethoxytitanium, n-decyltriethoxytitanium, n-didecyltriethoxytitanium, n-hexadecyltrimethoxytitanium, n-hexadecyltriethoxytitanium, and n-octadecyltrimethoxytitanium, and hydroxylates of the preceding.

The aluminate compound can be exemplified by methyltrimethoxyaluminum, dimethyltrimethoxyaluminum, methyltriethoxyaluminum, dimethyltriethoxyaluminum, ethyltrimethoxyaluminum, ethyltriethoxyaluminum, n-propyltrimethoxyaluminum, n-propyltriethoxyaluminum, n-butyltrimethoxyaluminum, n-butyltriethoxyaluminum, n-dibutyltrimethoxyaluminum, n-dibutyltriethoxyaluminum, n-dibutylethoxyaluminum, isobutyltrimethoxyaluminum, n-pentyltrimethoxyaluminum, n-pentyltriethoxyaluminum, hexyltrimethoxyaluminum, hexyltriethoxyaluminum, octyltrimethoxyaluminum, octyltriethoxyaluminum, n-decyltrimethoxyaluminum, n-decyltriethoxyaluminum, n-decylethoxyaluminum, n-didecylethoxyaluminum, n-hexadecyltrimethoxyaluminum, n-hexadecyltriethoxyaluminum, n-octadecyltrimethoxyaluminum, and hydroxylates of the preceding.

The zirconate compound can be exemplified by methyltrimethoxysirconium, dimethyltrimethoxysirconium, methyltriethoxysirconium, dimethyltriethoxysirconium, n-butyltrimethoxysirconium, n-dibutyltrimethoxysirconium,

13

n-butyltriethoxyzirconium, n-dibutylmethoxyzirconium, isobutyltrimethoxyzirconium, trimethylmethoxyzirconium, n-hexyltrimethoxyzirconium, n-octyltrimethoxyzirconium, n-octyltriethoxyzirconium, n-decyltrimethoxyzirconium, n-didecyldimethoxyzirconium, n-decyltriethoxyzirconium, n-didecyldiethoxyzirconium, n-hexadecyltrimethoxyzirconium, n-hexadecyltriethoxyzirconium, and n-octadecyltrimethoxyzirconium, and hydroxylates of the preceding.

A single one of the aforementioned silane compounds, titanate compounds, aluminate compounds, and zirconate compounds may be used by itself, or a plurality may be used in combination. When a plurality are used in combination, a separate treatment may be performed with each compound, or a simultaneous treatment may be carried out.

The amount of use of the surface treatment agent is not particularly limited and can be adjusted as appropriate within a range in which the effects of the present disclosure are not impaired.

The surface treatment agent may also be a surface treatment agent on which a hydrolysis treatment has been performed. Due to the execution of a hydrolysis treatment, adsorption occurs via hydrogen bonding with, e.g., the hydroxyl groups present on the inorganic fine particle surface, and heating and dehydration can then lead to the formation of strong chemical bonds. In addition, volatilization of the compound during heating can be suppressed through the formation of hydrogen bonds. Due to the occurrence of the chemical bonding, the treatment agent then does not detach from the inorganic fine particles during the toner production process and thus can be used without affecting the stability of toner production. Moreover, the low-temperature fixability and durability are improved because a high orientability is provided for the first monomer unit at the inorganic fine particle surface.

The amount of the surface treatment agent present on the inorganic fine particle surface can be determined by measuring the amount of carbon contained by the substrate, i.e., the inorganic fine particles, after treatment. The amount of carbon contained by the inorganic fine particles, expressed with reference to the inorganic fine particles, is preferably 0.30 mass % to 2.50 mass % and is more preferably 0.30 mass % to 2.00 mass %. Within this range, the surface treatment agent can be used without affecting the stability of toner production.

Among the preceding, compounds having the structure given by the following formula (3) are preferably used as the surface treatment agent. That is, the substrate has preferably been treated with a compound represented by the following formula (3). In other words, the inorganic fine particles are preferably the reaction product of the substrate and a compound represented by the following formula (3):



wherein R' represents an alkoxy group; m represents an integer of 1 to 3; Y' represents an alkyl group or a derivative thereof; and n represents an integer of 1 to 3; provided that m+n=4.

The number of carbons in the alkyl group encompassed by Y' is preferably 1 to 20 carbons, more preferably 4 to 16 carbons, and still more preferably 4 to 10 carbons. It is thought that, by having the number of carbons in the alkyl group be in the indicated range, a large interaction is then established between the alkyl group in the surface treatment agent and the monomer unit derived from the first polymerizable monomer and the crystallinity of the polymer A is

14

further increased. The heat-resistant storability and discharged paper adhesion behavior can be further enhanced as a consequence.

The alkyl group derivatives that can be represented by Y' can be specifically exemplified by the butylcyclopentyl group, butylcyclohexyl group, hexylcyclopentyl group, and hexylcyclohexyl group.

By having the surface treatment agent have the structure with formula (3), through control of the hydrolysis conditions self-condensation can be suppressed while also increasing the percentage hydrolysis, and a more uniform treatment of the inorganic fine particle surface can be achieved as a consequence. As a result, a uniform interaction occurs between the first monomer unit and the coating layer-bearing inorganic fine particles and a high crystallinity is achieved, a uniform crystalline state is established, and the discharged paper adhesion behavior and durability are further improved.

Methods for treating a metal oxide, e.g., magnetite, with a silane compound are provided below as examples. The following methods are examples and there is no limitation to or by these.

When the surface treatment is carried out by a wet method, a dispersion of the metal oxide dispersed in an aqueous medium is prepared. The pH of the obtained redispersion is adjusted to from 3.0 to 6.5; the alkoxy silane is gradually introduced; and dispersion to uniformity is carried out using, for example, a dispersing impeller. The liquid temperature of the dispersion at this time is preferably from 35° C. to 60° C. In general, hydrolysis of the alkoxy silane is facilitated at lower pH values and higher liquid temperatures.

Treatment using the silane compound may also be performed in the vapor phase. In a specific treatment method here, the silane compound is added by spraying while the untreated metal oxide is stirred with a Henschel mixer. This is followed by heating to a temperature at which the condensation reaction can proceed and then standing at quiescence and developing the condensation reaction of the silane compound while drying the metal oxide.

Fine particles having the silane compound chemically bonded to the metal oxide surface can be obtained using the methods described in the preceding.

It is also preferable that in the moisture adsorption/desorption curves for the inorganic fine particles, the following formulas (4) and (5) are satisfied:

$$1.5 \leq Z \leq 10.0 \quad (4)$$

$$Y - X \geq 0.10 \quad (5)$$

wherein X is an amount of moisture adsorption (mg/g) for the adsorption curve at 30.0° C. and 10% relative humidity, Y is an amount of moisture adsorption (mg/g) for the desorption curve at 30.0° C. and 10% relative humidity, and Z is an amount of moisture adsorption (mg/g) at 30.0° C. and 100% relative humidity.

By having Z in formula (4) be at least 1.5, even in a low-temperature, low-humidity environment the inorganic fine particles will adsorb an amount of moisture within a certain range, toner charge up can be suppressed, and the image quality can be further enhanced.

In addition, by having Z be not more than 10.0, the inorganic fine particles in the vicinity of the toner surface layer will not engage in excessive moisture adsorption in a high-temperature, high-humidity environment and an excess-

## 15

sive decline in the charge can be suppressed. The image quality in high-temperature, high-humidity environments can be improved as a result.

Z is more preferably 1.8 to 8.0 and is still more preferably 2.0 to 6.0.

By having Y-X satisfy formula (5), even in a low-temperature, low-humidity environment the inorganic fine particles in the toner surface layer can retain an appropriate amount of moisture and toner charge up can be suppressed. The image quality in low-temperature, low-humidity environments can be improved as a result. Y-X is more preferably at least 0.12 and is still more preferably at least 0.20.

The upper limit on Y-X is not particularly limited, but is preferably not more than 4.00, more preferably not more than 3.00, still more preferably not more than 2.00, and even more preferably not more than 0.40. Any combination may be used for the numerical value range for Y-X.

The method of producing inorganic fine particles that satisfy formula (4) and formula (5) is not particularly limited, but production may be carried out using, for example, the following production method.

The surface treatment can be carried out by a dry method using a wheel kneader or a mortar, for the purpose of causing the expression of a high hydrophobicity by uniformly reacting the surface treatment agent with the substrate particle surface, while at the same time causing an incomplete hydrophobing of the hydroxyl groups on the substrate particle surface in order to leave a portion thereof extant.

For example, a Mix Muller, Multimul, Stotz mill, back-flow kneader, or Eirich mill can be used as the wheel kneader, and the use of a Mix Muller is preferred.

Three actions, i.e., a compressive action, a shearing action, and a spatulation action, can be expressed when a wheel kneader or mortar is used.

The surface treatment agent present between substrate particles is pressed into the substrate surface through the compressive action and the adhesiveness and reactivity with the particle surface can then be increased. Shear force is applied to both the surface treatment agent and substrate through the shearing action and the surface treatment agent can then be smeared out and the substrate particles can be dispersed and disaggregated. Moreover, through the spatulation action, the surface treatment agent present on the substrate surface can be uniformly spread out as if spread with a spatula.

Through the continuous and repeated application of these three actions, the substrate is disaggregated and reaggregation is prevented, and the surface of individual particles can be surface-treated without bias while disaggregating into individual particles.

A stable treatment can be carried out by performing treatment using this method.

When the substrate is treated with the surface treatment agent using a wheel kneader or a mortar, a condition can be formed on the substrate particle surface in which a hydroxyl value that remains unreacted and portions that have reacted with the surface treatment agent are both present in alternation.

By establishing such a condition on the particle surface of the inorganic fine particles, a certain moisture adsorptivity can be provided while raising the hydrophobicity, and the Z value can be brought into the proper range and a large Y-X value can be established.

The toner particle contains a binder resin.

The binder resin contains a polymer A that includes a first monomer unit derived from a first polymerizable monomer

## 16

and a second monomer unit derived from a second polymerizable monomer that is different from the first polymerizable monomer.

In addition, the binder resin contains a polymer A that is 5 a polymer of a composition containing a first polymerizable monomer and a second polymerizable monomer that is different from the first polymerizable monomer.

The content of the first monomer unit in the polymer A, with reference to the total number of moles of all the 10 monomer units in the polymer A, is preferably 5.00 mol % to 60.00 mol %, more preferably 10.00 mol % to 60.00 mol %, and still more preferably 20.00 mol % to 40.00 mol %.

The content of the first polymerizable monomer in the 15 composition containing the first polymerizable monomer and the second polymerizable monomer, expressed with reference to the total number of moles of all the polymerizable monomer in the composition, is preferably 5.00 mol % to 60.00 mol %, more preferably 10.00 mol % to 60.00 mol %, and still more preferably 20.00 mol % to 40.00 mol %.

The content of the second monomer unit in the polymer 20 A, with reference to the total number of moles of all the monomer units in the polymer A, is preferably 20.00 mol % to 95.00 mol %, more preferably 40.00 mol % to 95.00 mol %, and still more preferably 40.00 mol % to 70.00 mol %.

The content of the second polymerizable monomer in the 25 composition, expressed with reference to the total number of moles of all the polymerizable monomer in the composition, is preferably 20.00 mol % to 95.00 mol %, more preferably 40.00 mol % to 95.00 mol %, and still more preferably 40.00 mol % to 70.00 mol %.

Through the interaction between the polymer A and the 30 inorganic fine particles, a higher crystallinity than heretofore is obtained for toner that contains the coating layer-bearing inorganic fine particles and that has a content of first monomer unit in the polymer A and a content of first polymerizable monomer in the composition in the aforementioned ranges. As a result, the sharp melt property and 35 elasticity of the toner are improved and an excellent low-temperature fixability, durability, heat-resistant storability, and discharged paper adhesion behavior are established.

When the content of the second monomer unit in the 40 polymer A and the content of the second polymerizable monomer in the composition are in the aforementioned ranges, the polymer A can exhibit an improved elasticity at around room temperature while retaining a sharp melt property, and a toner having an excellent low-temperature fixability and an excellent durability is then provided. In addition, the inhibition of the crystallization of the first monomer unit in the polymer A is suppressed and the melting point can also be maintained. A satisfactory interaction between the second monomer unit and the high-polarity segment of the inorganic fine particle surface is also 45 obtained and a good discharged paper adhesion behavior is obtained.

The first polymerizable monomer is at least one selected from the group consisting of (meth)acrylate esters having an alkyl group having 18 to 36 carbons.

The (meth)acrylate esters having an alkyl group having 18 50 to 36 carbons can be exemplified by (meth)acrylate esters having a linear alkyl group having 18 to 36 carbons [e.g., stearyl (meth)acrylate, nonadecyl (meth)acrylate, eicosyl (meth)acrylate, heneicosyl (meth)acrylate, behenyl (meth)acrylate, lignoceryl (meth)acrylate, ceryl (meth)acrylate, 55 octacosyl (meth)acrylate, myricyl (meth)acrylate, and dotriacontanyl (meth)acrylate] and by (meth)acrylate esters

having a branched alkyl group having 18 to 36 carbons [e.g., 2-decytetradecyl (meth)acrylate].

Among the preceding, at least one selected from the group consisting of (meth)acrylate esters having a linear alkyl group having 18 to 36 carbons is preferred from the standpoint of the heat-resistant storability of the toner. At least one selected from the group consisting of (meth)acrylate esters having a linear alkyl group having 18 to 30 carbons is more preferred. At least one selected from the group consisting of linear stearyl (meth)acrylate and behenyl (meth)acrylate is still more preferred.

A single first polymerizable monomer may be used by itself or two or more may be used in combination.

The second polymerizable monomer can be exemplified by those polymerizable monomers, among the polymerizable monomers provided below, that satisfy formula (1) or formula (2). The second polymerizable monomer preferably has an ethylenically unsaturated bond and more preferably has one ethylenically unsaturated bond. A single second polymerizable monomer may be used by itself or two or more may be used in combination.

Nitrile group-bearing monomers can be exemplified by acrylonitrile and methacrylonitrile.

Examples of hydroxy group-bearing monomers are 2-hydroxyethyl (meth)acrylate and 2-hydroxypropyl (meth)acrylate.

Examples of amide group-bearing monomers are acrylamide and monomers provided by reaction by a known method between an amine having 1 to 30 carbons and a carboxylic acid having 2 to 30 carbons and containing an ethylenically unsaturated bond (e.g., acrylic acid, methacrylic acid).

Urethane group-bearing monomers can be exemplified by monomers provided by the reaction by a known method of an alcohol having 2 to 22 carbons and an ethylenically unsaturated bond (e.g., 2-hydroxyethyl methacrylate and vinyl alcohol) with an isocyanate having 1 to 30 carbons [e.g., monoisocyanate compounds (e.g., benzenesulfonyl isocyanate, tosyl isocyanate, phenyl isocyanate, p-chlorophenyl isocyanate, butyl isocyanate, hexyl isocyanate, t-butyl isocyanate, cyclohexyl isocyanate, octyl isocyanate, 2-ethylhexyl isocyanate, dodecyl isocyanate, adamantyl isocyanate, 2,6-dimethylphenyl isocyanate, 3,5-dimethylphenyl isocyanate, and 2,6-dipropylphenyl isocyanate), aliphatic diisocyanate compounds (e.g., trimethylene diisocyanate, tetramethylene diisocyanate, hexamethylene diisocyanate, pentamethylene diisocyanate, 1,2-propylene diisocyanate, 1,3-butylene diisocyanate, dodecamethylene diisocyanate, and 2,4,4-trimethylhexamethylene diisocyanate), alicyclic diisocyanate compounds (e.g., 1,3-cyclopentene diisocyanate, 1,3-cyclohexane diisocyanate, 1,4-cyclohexane diisocyanate, isophorone diisocyanate, hydrogenated diphenylmethane diisocyanate, hydrogenated xylylene diisocyanate, hydrogenated tolylene diisocyanate, and hydrogenated tetramethylxylylene diisocyanate), and aromatic diisocyanate compounds (e.g., phenylene diisocyanate, 2,4-tolylene diisocyanate, 2,6-tolylene diisocyanate, 2,2'-diphenylmethane diisocyanate, 4,4'-diphenylmethane diisocyanate, 4,4'-toluidine diisocyanate, 4,4'-diphenyl ether diisocyanate, 4,4'-diphenyl diisocyanate, 1,5-naphthalene diisocyanate, and xylylene diisocyanate)], and

by monomers provided by the reaction by a known method between an alcohol having 1 to 26 carbons (e.g., methanol, ethanol, propanol, isopropyl alcohol, butanol, t-butyl alcohol, pentanol, heptanol, octanol, 2-ethylhexanol, nonanol, decanol, undecyl alcohol, lauryl alcohol, dodecyl alcohol, myristyl alcohol, pentadecyl alcohol, cetanol, hept-

tadecanol, stearyl alcohol, isostearyl alcohol, elaidyl alcohol, oleyl alcohol, linoleyl alcohol, linolenyl alcohol, nonadecyl alcohol, heneicosanol, behenyl alcohol, erucyl alcohol) and an isocyanate having 2 to 30 carbons and containing an ethylenically unsaturated bond [e.g., 2-isocyanatoethyl (meth)acrylate, 2-(O-[1'-methylpropylideneamino]carboxyamino)ethyl (meth)acrylate, 2-[(3,5-dimethylpyrazolyl)carbonylamino]ethyl (meth)acrylate, and 1,1-(bis(meth)acryloyloxyethyl)ethyl isocyanate].

Examples of urea group-bearing monomers are monomers provided by the reaction by a known method of an amine having 3 to 22 carbons [e.g., primary amines (normal-butylamine, t-butylamine, propylamine, and isopropylamine), secondary amines (e.g., di-normal-ethylamine, di-normal-propylamine, and di-normal-butylamine), aniline, and cyclohexylamine] with an isocyanate having 2 to 30 carbons and an ethylenically unsaturated bond.

Examples of carboxy group-bearing monomers are methacrylic acid, acrylic acid, and 2-carboxyethyl (meth)acrylate.

Among the preceding, the use of monomer bearing a nitrile group, amide group, urethane group, hydroxy group, or urea group is preferred. The second polymerizable monomer is more preferably a monomer that has an ethylenically unsaturated bond and at least one functional group selected from the group consisting of the nitrile group, amide group, hydroxy group, urethane group, and urea group.

The presence of these facilitates a high melting point for the polymer A and facilitates an improved heat-resistant storability. In addition, the elasticity around room temperature is increased and improvement in the durability is facilitated.

A vinyl ester, e.g., vinyl acetate, vinyl propionate, vinyl butyrate, vinyl caproate, vinyl caprylate, vinyl caprate, vinyl laurate, vinyl myristate, vinyl palmitate, vinyl stearate, vinyl pivalate, and vinyl octanoate, is also preferably used for the second polymerizable monomer. Vinyl esters are nonconjugated monomers, and the reactivity with the first polymerizable monomer is readily appropriately maintained. It is thought that as a consequence the formation is facilitated of a condition in which monomer units derived from the first polymerizable monomer are bonded in aggregate in the polymer A and the crystallinity of the polymer A is increased and the coexistence of the low-temperature fixability and heat-resistant storability is further facilitated.

In addition, the second polymerizable monomer is preferably at least one selected from the group consisting of the following formulas (E) and (F):



19

in formula (E), X represents a single bond or an alkylene group having 1 to 6 carbons;

R<sup>8</sup> represents a nitrile group (—C≡N),

amide group (—C(=O)NHR<sup>11</sup>, wherein R<sup>11</sup> is a hydrogen atom or an alkyl group having 1 to 4 carbons), hydroxy group,

—COOR<sup>12</sup>, wherein R<sup>12</sup> is an alkyl group having 1 to 6 (preferably 1 to 4) carbons or a hydroxyalkyl group having 1 to 6 (preferably 1 to 4) carbons,

urethane group (—NHCOOR<sup>13</sup>, wherein R<sup>13</sup> is an alkyl group having 1 to 4 carbons,

urea group (—NH—C(=O)—N(R<sup>14</sup>)<sub>2</sub>, wherein each R<sup>14</sup> is independently a hydrogen atom or an alkyl group having 1 to 6 (preferably 1 to 4) carbons),

—COO(CH<sub>2</sub>)<sub>2</sub>NHCOOR<sup>15</sup>, wherein R<sup>15</sup> is an alkyl group having 1 to 4 carbons, or —COO(CH<sub>2</sub>)<sub>2</sub>—NH—C(=O)—N(R<sup>16</sup>)<sub>2</sub>, wherein each R<sup>16</sup> is independently a hydrogen atom or an alkyl group having 1 to 6 (preferably 1 to 4) carbons; and

R<sup>10</sup> represents a hydrogen atom or methyl group, and in formula (F), R<sup>9</sup> represents an alkyl group having 1 to 4 carbons and

R<sup>10</sup> represents a hydrogen atom or a methyl group.

In addition, the second polymerizable monomer is preferably at least one selected from the group consisting of the following formulas (E) and (F):



in formula (E), X represents a single bond or an alkylene group having 1 to 6 carbons;

R<sup>8</sup> represents a nitrile group (—C≡N),

amide group (—C(=O)NHR<sup>11</sup>, wherein R<sup>11</sup> is a hydrogen atom or an alkyl group having 1 to 4 carbons), hydroxy group,

—COOR<sup>12</sup>, wherein R<sup>12</sup> is an alkyl group having 1 to 6 (preferably 1 to 4) carbons or a hydroxyalkyl group having 1 to 6 (preferably 1 to 4) carbons,

urea group (—NH—C(=O)—N(R<sup>14</sup>)<sub>2</sub>, wherein each R<sup>14</sup> is independently a hydrogen atom or an alkyl group having 1 to 6 carbons),

—COO(CH<sub>2</sub>)<sub>2</sub>NHCOOR<sup>15</sup>, wherein R<sup>15</sup> is an alkyl group having 1 to 4 carbons, or —COO(CH<sub>2</sub>)<sub>2</sub>—NH—C(=O)—N(R<sup>16</sup>)<sub>2</sub>, wherein each R<sup>16</sup> is independently a hydrogen atom or an alkyl group having 1 to 6 (preferably 1 to 4) carbons; and

R<sup>10</sup> represents a hydrogen atom or methyl group, and in formula (F), R<sup>9</sup> represents an alkyl group having 1 to 4 carbons and

R<sup>10</sup> represents a hydrogen atom or a methyl group.

The polymer A is preferably a vinyl polymer. Vinyl polymers can be exemplified by polymers from monomers

20

that contain an ethylenically unsaturated bond. The ethylenically unsaturated bond denotes a carbon-carbon double bond capable of undergoing radical polymerization and can be exemplified by the vinyl group, propenyl group, acryloyl group, and methacryloyl group.

The polymer A may contain, within a range that preserves the aforementioned molar ratios for the first monomer unit derived from the first polymerizable monomer and the second monomer unit derived from the second polymerizable monomer, a third monomer unit derived from a third polymerizable monomer that is different from the first polymerizable monomer and different from the second polymerizable monomer.

In addition, the composition containing the first polymerizable monomer and the second polymerizable monomer different from the first polymerizable monomer, may contain, within a range that preserves the contents in the composition of the first polymerizable monomer and the second polymerizable monomer, a third polymerizable monomer different from the first polymerizable monomer and different from the second polymerizable monomer.

In these cases, where  $SP_{31}$  (J/cm<sup>3</sup>)<sup>0.5</sup> designates the SP value of the third monomer unit derived from the third polymerizable monomer, the relationship in the following formula (7) is preferably satisfied:

$$0.00 < (SP_{31} - SP_{11}) < 3.00 \quad (7)$$

In addition, where  $SP_{32}$  (J/cm<sup>3</sup>)<sup>0.5</sup> designates the SP value of the third polymerizable monomer, the relationship in the following formula (8) is preferably satisfied:

$$0.00 < (SP_{32} - SP_{12}) < 0.60 \quad (8)$$

Those monomers, among the monomers provided above as examples of the second polymerizable monomer, that satisfy formula (7) or formula (8) may be used as the third polymerizable monomer.

The monomer unit derived from the third polymerizable monomer applies to all monomer units having an  $SP_{31}$  that satisfies formula (7) with respect to  $SP_{11}$ . Similarly, the third polymerizable monomer applies to all polymerizable monomers having an  $SP_{32}$  that satisfies formula (8) with respect to  $SP_{12}$ .

That is, when the third polymerizable monomer is two or more species of polymerizable monomers,  $SP_{31}$  represents the SP value of the monomer unit derived from each polymerizable monomer and  $SP_{31} - SP_{11}$  is determined for the monomer unit derived from each third polymerizable monomer. Similarly,  $SP_{32}$  represents the SP value of each polymerizable monomer and  $SP_{32} - SP_{12}$  is determined for each third polymerizable monomer.

The following, for example, can be used as the third polymerizable monomer:

styrene and derivatives thereof, e.g., styrene and o-methylstyrene, and (meth)acrylate esters such as n-butyl (meth)acrylate, t-butyl (meth)acrylate, and 2-ethylhexyl (meth)acrylate.

Styrene, methyl methacrylate, and methyl acrylate are preferred among the aforementioned third polymerizable monomers. Their use facilitates improvements in the durability.

These monomers do not contain a polar group and thus have low SP values, making it difficult for them to satisfy formula (1) or formula (2). However, when they do satisfy formula (1) or formula (2), they can be used as the second polymerizable monomer.

A charge control agent may be used in the toner particle in order to maintain a stable charging performance for the toner regardless of the environment.

Negative-charging charge control agents can be exemplified by monoazo metal compounds; acetylacetone-metal compounds; metal compounds of aromatic oxycarboxylic acids, aromatic dicarboxylic acids, oxycarboxylic acids, and dicarboxylic acids; aromatic oxycarboxylic acids, aromatic monocarboxylic acids, and aromatic polycarboxylic acids and their metal salts, anhydrides, and esters; phenol derivatives such as bisphenol; urea derivatives; metal-containing salicylic acid compounds; metal-containing naphthoic acid compounds; boron compounds; quaternary ammonium salts; calixarene; and resin-type charge control agents.

Positive-charging charge control agents can be exemplified by nigrosine and modifications of nigrosine by, e.g., fatty acid metal salts; guanidine compounds; imidazole compounds; quaternary ammonium salts such as the tributylbenzylammonium salt of 1-hydroxy-4-naphthosulfonic acid and tetrabutylammonium tetrafluoroborate, and their onium salt analogues, e.g., phosphonium salts, and their lake pigments; triphenylmethane dyes and their lake pigments (the lake agent can be exemplified by phosphotungstic acid, phosphomolybdic acid, phosphotungstomolybdic acid, tannic acid, lauric acid, gallic acid, ferricyanide, and ferrocyanide); metal salts of higher fatty acids; diorganotin oxides such as dibutyltin oxide, diocetyltin oxide, and dicyclohexyltin oxide; diorganotin borates such as dibutyltin borate, diocetyltin borate, and dicyclohexyltin borate; and resin-type charge control agents.

The content of the charge control agent, per 100 mass parts of the binder resin, is preferably 0.01 mass parts to 10 mass parts and more preferably 0.03 to 8 mass parts. A single one of these charge control agents may be used by itself or two or more may be used in combination.

The toner particle may contain a release agent.

The release agent can be exemplified by the following: waxes in which the main component is a fatty acid ester, e.g., carnauba wax and montanic acid ester wax; waxes provided by the partial or complete deacidification of the acid component from a fatty acid ester, e.g., deacidified carnauba wax; hydroxyl group-containing methyl ester compounds obtained by, e.g., the hydrogenation of plant oils; saturated fatty acid monoesters, e.g., stearyl stearate and behenyl behenate; diesters between a saturated aliphatic dicarboxylic acid and a saturated aliphatic alcohol, e.g., dibehenyl sebacate, distearyl dodecanedioate, and distearyl octadecanedioate; diesters between a saturated aliphatic diol and a saturated fatty acid, e.g., nonanediol dibehenate and dodecanediol distearyl; aliphatic hydrocarbon waxes such as low molecular weight polyethylene, low molecular weight polypropylene, microcrystalline wax, paraffin wax, and Fischer-Tropsch wax; the oxides of aliphatic hydrocarbon waxes, e.g., oxidized polyethylene wax, and their block copolymers; waxes provided by grafting an aliphatic hydrocarbon wax using a vinyl monomer such as styrene or acrylic acid; saturated straight-chain fatty acids such as palmitic acid, stearic acid, and montanic acid; unsaturated fatty acids such as brassidic acid, eleostearic acid, and parinaric acid; saturated alcohols such as stearyl alcohol, aralkyl alcohols, behenyl alcohol, carnaubyl alcohol, ceryl alcohol, and melissyl alcohol; polyhydric alcohols such as sorbitol; fatty acid amides such as linoleamide, oleamide, and lauramide; saturated fatty acid bisamides such as methylenebisstearamide, ethylenebiscapramide, ethylenebislauroamide, and hexamethylenebisstearamide; unsaturated fatty acid amides such as ethylenebisoleamide, hexamethylenebisoleamide,

N,N'-dioleyladipamide, and N,N'-dioleylsebacamide; aromatic bisamides such as m-xylenebisstearamide and N,N'-distearylisophthalamide; fatty acid metal salts (generally known as metal soaps) such as calcium stearate, calcium laurate, zinc stearate, and magnesium stearate; and long-chain alkyl alcohols or long-chain alkylcarboxylic acids having at least 12 carbons.

The content of the release agent in the toner particle is preferably 1.0 mass % to 30.0 mass % and is more preferably 2.0 mass % to 25.0 mass %.

The weight-average molecular weight (Mw) of the tetrahydrofuran (THF)-soluble matter of the polymer A, as measured by gel permeation chromatography (GPC), is preferably 10,000 to 200,000 and more preferably 20,000 to 150,000.

Maintenance of the elasticity at around room temperature is facilitated by having the weight-average molecular weight (Mw) be in the indicated range. In addition, the melting point of the polymer A is preferably 50° C. to 80° C. and is more preferably 53° C. to 70° C. Additional improvements in the low-temperature fixability and heat-resistant storability are obtained by having the melting point be in the indicated range.

The melting point of the polymer A can be adjusted through, for example, the type and amount of the first polymerizable monomer that is used and the type and amount of the second polymerizable monomer that is used.

The content of the polymer A in the binder resin is preferably at least 50.0 mass % and is more preferably 80.0 mass % to 100.0 mass %. Even more preferably the binder resin is the polymer A. Retention of the sharp melt property by the toner is facilitated and the low-temperature fixability is enhanced by having the polymer A content in the binder resin be in the indicated range.

Resins that may be used for the binder resin in addition to the polymer A can be exemplified by the heretofore known vinyl resins, polyester resins, polyurethane resins, epoxy resins, and so forth. Vinyl resins, polyester resins, and polyurethane resins are preferred thereamong from the standpoint of the electrophotographic characteristics.

The polymerizable monomers that can be used for the vinyl resins can be exemplified by the polymerizable monomers that can be used for the above-described first polymerizable monomer, second polymerizable monomer, and third polymerizable monomer. A combination of two or more species may be used on an optional basis.

The polyester resin can be obtained by the reaction of an at least dibasic polybasic carboxylic acid with a polyhydric alcohol.

The following compounds are examples of polybasic carboxylic acids: dibasic acids such as succinic acid, adipic acid, sebatic acid, phthalic acid, isophthalic acid, terephthalic acid, malonic acid, and dodecenylysuccinic acid, and their anhydrides and lower alkyl esters; aliphatic unsaturated dicarboxylic acids such as maleic acid, fumaric acid, itaconic acid, and citraconic acid; as well as 1,2,4-benzenetricarboxylic acid and 1,2,5-benzenetricarboxylic acid and their anhydrides and lower alkyl esters. A single one of these may be used by itself or two or more may be used in combination.

The polyhydric alcohol can be exemplified by the following compounds: alkylene glycols (ethylene glycol, 1,2-propylene glycol, and 1,3-propylene glycol), alkylene ether glycols (polyethylene glycol and polypropylene glycol), alicyclic diols (1,4-cyclohexanedimethanol), bisphenols (bisphenol A), and alkylene oxide (ethylene oxide and propylene oxide) adducts on alicyclic diols. The alkyl moi-

ties in the alkylene glycols and alkylene ether glycols may be straight chain or branched chain. Additional examples are glycerol, trimethylolethane, trimethylolpropane, and pentaerythritol. A single one of these may be used by itself or two or more may be used in combination.

As necessary, a monobasic acid such as acetic acid or benzoic acid and a monohydric alcohol such as cyclohexanol or benzyl alcohol may also be used for the purpose of adjusting the acid value or hydroxyl value.

There are no particular limitations on the method of producing the polyester resin, but, for example, a transesterification method or direct polycondensation method, as such or in combination, may be used.

The polyurethane resin is considered in the following. The polyurethane resin is the reaction product of a diol with a substance that contains the diisocyanate group, and resins having various functionalities can be obtained by adjusting the diol and diisocyanate.

The diisocyanate component can be exemplified by the following: aromatic diisocyanates having from 6 to 20 carbons (excluding the carbon in the NCO group, the same applies in the following), aliphatic diisocyanates having from 2 to 18 carbons, and alicyclic diisocyanates having from 4 to 15 carbons, as well as modifications of these diisocyanates (modifications that contain the urethane group, carbodiimide group, allophanate group, urea group, biuret group, uretdione group, uretoimine group, isocyanurate group, or oxazolidone group, also referred to herebelow as "modified diisocyanate") and mixtures of two or more of the preceding.

The following are examples of the aromatic diisocyanates: m- and/or p-xylylene diisocyanate (XDI) and  $\alpha,\alpha,\alpha'$ ,  $\alpha'$ -tetramethylxylylene diisocyanate.

The following are examples of the aliphatic diisocyanates: ethylene diisocyanate, tetramethylene diisocyanate, hexamethylene diisocyanate (HDI), and dodecamethylene diisocyanate.

The following are examples of alicyclic diisocyanates: isophorone diisocyanate (IPDI), dicyclohexylmethane-4,4'-diisocyanate, cyclohexylene diisocyanate, and methylcyclohexylene diisocyanate.

Preferred among the preceding are aromatic diisocyanates having from 6 to 15 carbons, aliphatic diisocyanates having from 4 to 12 carbons, and alicyclic diisocyanates having from 4 to 15 carbons, wherein XDI, IPDI, and HDI are particularly preferred. A trifunctional or higher functional isocyanate compound may also be used in addition to the diisocyanate component.

The same dihydric alcohols usable for the polyester resin as described above can be adopted for the diol component that can be used for the polyurethane resin.

The toner particle may contain a colorant. The colorant can be exemplified by known organic pigments, organic dyes, and inorganic pigments, and black colorants can be exemplified by carbon black and magnetic bodies. In addition to these, those colorants conventionally used in toners may be used.

The inorganic fine particles described in the preceding may also be used as the colorant.

The toner particle configuration may be that of a core/shell structure in which a shell is formed on the surface of a core particle.

The method for forming this core/shell structure is not particularly limited; however, for example, a polymer layer functioning as the shell may be formed by the suspension polymerization, in the presence of a core particle, of polymerizable monomer for the shell.

Monomer that forms a polymer having a glass transition temperature above 70° C., e.g., styrene, methyl methacrylate, and so forth, is preferably used as the polymerizable monomer for shell formation, and a single one of these or a combination of two or more may be used. Methyl methacrylate is more preferred.

In order to improve toner storability, the glass transition temperature of the polymer obtained from the polymerizable monomer for shell formation is preferably 50° C. to 120° C., more preferably 60° C. to 110° C., and still more preferably 70° C. to 105° C.

In addition, from the standpoint of heat resistance the shell may contain a thermosetting resin.

This thermosetting resin can be exemplified by the following:

melamine resins, urea resins, sulfonamide resins, glyoxal resins, guanamine resins, and aniline resins and derivatives of these resins;

20 polyimide resins; maleimide polymers from, e.g., bismaleimide, aminobismaleimide, or bismaleimide triazine; and resins (referred to below as aminoaldehyde resins) produced by the polycondensation of an amino group-containing compound and an aldehyde (for example, formaldehyde) 25 as well as derivatives of aminoaldehyde resins.

The melamine resins are the polycondensates of melamine with formaldehyde. The urea resins are the polycondensates of urea and formaldehyde. The glyoxal resins are the polycondensates of formaldehyde with the reaction product of glyoxal and urea. The glyoxal resin is preferably dimethyloldihydroxyethyleneurea (DMDHEU).

The crosslinking and curing function of the thermosetting resin can be improved by the presence of the element nitrogen in the thermosetting resin. In order to increase the 35 reactivity of the thermosetting resin, the content of the element nitrogen is preferably adjusted to from 40 mass % to 55 mass % for melamine resins, to about 40 mass % for urea resins, and to about 15 mass % for glyoxal resins.

At least one thermosetting monomer selected from the 40 group consisting of methylolmelamine, melamine, methyloated urea, urea, benzoguanamine, acetoguanamine, and spiroguanamine can advantageously be used in the preparation of the thermosetting resin contained in the shell.

A curing agent or reaction promoter may be used for shell 45 formation, and a polymer in which a plurality of functional groups are combined may be used for shell formation. In addition, the water-resistance of the shell can be improved using an acrylsilicone resin (graft polymer).

The thickness of the shell is preferably not more than 20 50 nm and is more preferably 3 nm to 20 nm. Shell formation is preferably carried out in an aqueous medium, and the material of the shell preferably has water solubility.

In order to form the shell with the thermosetting resin, preferably the core particle has an anionic character and the 55 shell has a cationic character. By having the core particle have an anionic character, the cationic shell material can then be attracted to the core particle surface during shell formation.

Considered in greater detail, for example, the shell material, being positively charged in the aqueous medium, is electrically attracted to the core particle, which is negatively charged in the aqueous medium, and the shell layer is then formed on the core particle surface by in-situ polymerization. By proceeding in this manner, the formation of a uniform shell on the core particle surface is facilitated even without inducing an excessive dispersion of the core particles in the aqueous medium using a dispersing agent.

The toner preferably contains an external additive in order to improve the charge stability, developing performance, flowability, and durability. This external additive can be exemplified by inorganic fine particles, e.g., silica fine particles and metal oxide fine particles (e.g., alumina fine particles, titanium oxide fine particles, magnesium oxide fine particles, zinc oxide fine particles, strontium titanate fine particles, and barium titanate fine particles).

Organic fine particles including, e.g., a vinyl resin, silicone resin, or melamine resin, and organic/inorganic composite fine particles may also be used.

The content of the external additive, per 100.0 mass parts of the toner particle, is preferably from 0.1 mass parts to 4.0 mass parts and is more preferably from 0.2 mass parts to 3.5 mass parts.

The toner particle may be produced by any heretofore known method, i.e., a suspension polymerization method, emulsion aggregation method, dissolution suspension method, or pulverization method, as long as the toner particle falls within the range of the herein described constitution; however, production by the suspension polymerization method is preferred. That is, the toner particle is preferably a suspension-polymerized toner particle.

When the toner particle is produced by the suspension polymerization method, the inorganic fine particles can be segregated to the vicinity of the toner surface layer through selection, so as to satisfy the conditions of the present disclosure, of the particle diameter and content of the inorganic fine particles, the type and amount of addition of the surface treatment agent used to treat the inorganic fine particles, and the treatment method with the surface treatment agent. As a result, a high crystallinity by the crystalline resin is established in the vicinity of the surface layer and the low-temperature fixability and durability are then further improved.

For example, a polymerizable monomer composition is obtained by mixing the polymerizable monomer that will produce the binder resin including the polymer A, with the inorganic fine particles and optional other additives such as release agent, charge control agent, and so forth. This polymerizable monomer composition is then added to an aqueous medium (optionally containing a dispersion stabilizer). Particles of the polymerizable monomer composition are formed in the aqueous medium and toner particles can then be obtained by polymerizing the polymerizable monomer in these particles.

The methods used to measure the properties involved with the present disclosure are described in the following.

Method for Measuring the Contents in the Polymer A of the Monomer Units Derived from the Various Polymerizable Monomers

The contents in the polymer A of the monomer units derived from the various polymerizable monomers are measured by  $^1\text{H-NMR}$  using the following conditions.

measurement instrument: JNM-EX400 FT-NMR instrument (JEOL Ltd.)

measurement frequency: 400 MHz

pulse condition: 5.0  $\mu\text{s}$

frequency range: 10,500 Hz

number of accumulations: 64

measurement temperature: 30° C.

sample: Preparation is carried out by introducing 50 mg of

the measurement sample into a sample tube having an internal diameter of 5 mm; adding deuteriochloroform ( $\text{CDCl}_3$ ) as solvent; and dissolving in a 40° C. thermostat.

From among the peaks assigned to the constituent components of the monomer unit derived from the first polymerizable monomer in the resulting  $^1\text{H-NMR}$  chart, a peak is selected that is independent from the peaks assigned to the constituent components for otherwise derived monomer units, and the integration value  $S_1$  of this peak is calculated.

Similarly, from among the peaks assigned to the constituent components of the monomer unit derived from the second polymerizable monomer, a peak is selected that is independent from the peaks assigned to the constituent components for otherwise derived monomer units, and the integration value  $S_2$  of this peak is calculated.

When a third polymerizable monomer has been used, from among the peaks assigned to the constituent components of the monomer unit derived from the third polymerizable monomer, a peak is selected that is independent from the peaks assigned to the constituent components for otherwise derived monomer units, and the integration value  $S_3$  of this peak is calculated.

The content of monomer unit derived from the first polymerizable monomer is determined as follows using the integration values  $S_1$ ,  $S_2$ , and  $S_3$ .  $n_1$ ,  $n_2$ , and  $n_3$  are the number of hydrogens in the constituent component to which the peak of interest for the particular segment is assigned.

$$\text{content (mol \%)} \text{ of monomer unit derived from the first polymerizable monomer} = \left\{ \frac{(S_1/n_1)}{(S_1/n_1) + (S_2/n_2) + (S_3/n_3)} \right\} \times 100$$

The content of the monomer unit derived from the second polymerizable monomer and the content of the monomer unit derived from the third polymerizable monomer are similarly determined as follows.

$$\text{content (mol \%)} \text{ of monomer unit derived from the second polymerizable monomer} = \left\{ \frac{(S_2/n_2)}{(S_1/n_1) + (S_2/n_2) + (S_3/n_3)} \right\} \times 100$$

$$\text{content (mol \%)} \text{ of monomer unit derived from the third polymerizable monomer} = \left\{ \frac{(S_3/n_3)}{(S_1/n_1) + (S_2/n_2) + (S_3/n_3)} \right\} \times 100$$

When polymerizable monomer that does not contain the hydrogen atom in a constituent component other than the vinyl group is used for the polymer A,  $^{13}\text{C}$  is used for the measurement atomic nucleus using  $^{13}\text{C-NMR}$ ; measurement is performed in single pulse mode; and the calculation is carried out proceeding as with the  $^1\text{H-NMR}$ .

In addition, when the toner particle is produced by suspension polymerization, the peaks for the release agent and other resins may overlap and an independent peak may not be observed. Due to this, it may then not be possible in some instances to calculate the contents of the monomer units derived from the various polymerizable monomers in the polymer A. When this is the case, a polymer A' is produced by the same suspension polymerization, but without using the inorganic fine particles, release agent, and other resins, and the analysis can then be performed taking the polymer A' as the polymer A.

Method for Calculating SP Values

$\text{SP}_{12}$ ,  $\text{SP}_{22}$ , and  $\text{SP}_{32}$  are determined proceeding as follows using the calculation method proposed by Fedors.

For each of the polymerizable monomers, the energy of vaporization ( $\Delta\text{ei}$ ) (cal/mol) and the molar volume ( $\Delta\text{vi}$ ) ( $\text{cm}^3/\text{mol}$ ) are determined from the tables given in "Polym. Eng. Sci., 14(2), 147-154 (1974)" for the atoms or atomic groups in the molecular structure, and  $(4.184 \times \sum \Delta\text{ei} / \sum \Delta\text{vi})^{0.5}$  is used for the SP value ( $\text{J/cm}^3)^{0.5}$ .

$\text{SP}_{11}$ ,  $\text{SP}_{21}$ , and  $\text{SP}_{31}$ , on the other hand, are determined by this same calculation method for the atoms or atomic

groups in the molecular structure residing in the state provided by cleavage of the double bond in the polymerizable monomer due to polymerization.

Method for Measuring the Weight-Average Molecular Weight (Mw) of the Polymer A

The weight-average molecular weight (Mw) of the tetrahydrofuran (THF)-soluble matter in the polymer A is measured using gel permeation chromatography (GPC) as follows.

First, the sample is dissolved in tetrahydrofuran (THF) at room temperature for 24 hours. The obtained solution is filtered using a "Sample Pretreatment Cartridge" (Tosoh Corporation) solvent-resistant membrane filter having a pore diameter of 0.2  $\mu$ m to obtain a sample solution. The sample solution is adjusted to a concentration of THF-soluble component of 0.8 mass %. Measurement is carried out under the following conditions using this sample solution.

instrument: HLC8120 GPC (detector: RI) (Tosoh Corporation)

column: 7-column train of Shodex KF-801, 802, 803, 804, 805, 806, and 807 (Showa Denko Kabushiki Kaisha)

eluent: tetrahydrofuran (THF)

flow rate: 1.0 mL/min

oven temperature: 40.0°C.

sample injection amount: 0.10 mL

A molecular weight calibration curve constructed using polystyrene resin standards (product name "TSK Standard Polystyrene F-850, F-450, F-288, F-128, F-80, F-40, F-20, F-10, F-4, F-2, F-1, A-5000, A-2500, A-1000, A-500", Tosoh Corporation) is used to determine the molecular weight of the sample.

Method for Measuring the Melting Point of the Polymer A

The melting point of the polymer A is measured using the following conditions and a DSC Q1000 (TA Instruments). ramp rate: 10° C./min

measurement start temperature: 20° C.

measurement end temperature: 180° C.

The melting points of indium and zinc are used for temperature correction in the instrument detection section, and the heat of fusion of indium is used for correction of the amount of heat.

Specifically, 5 mg of the sample is exactly weighed out and introduced into an aluminum pan and differential scanning calorimetric measurement is carried out. An empty silver pan is used for reference.

The peak temperature of the maximum endothermic peak in the first heating step is taken to be the melting point (°C.).

When a plurality of peaks are present, the maximum endothermic peak is taken to be the peak having the largest endothermic quantity.

Analysis of the Structure of the Coating Layer on the Inorganic Fine Particles

The measurement is carried out using the following conditions and time-of-flight secondary ion mass spectrometry (TOF-SIMS). A TRIFT-IV from ULVAC-PHI, Inc. is used as the instrumentation.

sample preparation: the inorganic fine particles are attached to an indium sheet

sample pretreatment: none

primary ion: Au ion

acceleration voltage: 30 kV

charge neutralization mode: ON

measurement mode: Negative

raster: 100  $\mu$ m

The structure of the inorganic fine particle surface can be elucidated by the presence/absence of peaks that represent

bonding between the surface treatment agent and inorganic elements present in the inorganic fine particles.

Method for Measuring the Amount of Treatment Agent on the Inorganic Fine Particle Surface

5 The amount of carbon per unit weight is measured using a carbon/sulfur analyzer (EMIA-320V) from Horiba, Ltd. The amount of carbon provided by this measurement is taken to be the amount of treatment agent (mass %) at the inorganic fine particle surface. The measurement is carried out using 0.20 g for the amount of introduction of the inorganic fine particles and a mixture of tungsten and tin for the combustion improver.

Method for Measuring the Content of Inorganic Fine Particles in the Toner

15 The measurement is carried out as follows using a "product name: TGA7, from PerkinElmer Inc." thermal analyzer. The toner is heated from normal temperature to 900° C. under a nitrogen atmosphere at a ramp rate of 25° C./minute. The mass loss in mass % between 100° C. and 750° C. is taken to be the amount of binder resin, and the remaining mass is taken to be approximately equal to the amount of the inorganic fine particles.

20 When the toner has an external additive, measurement of the inorganic fine particle content is carried out after the external additive has been removed using the following methods.

For the Case of a Magnetic Toner

25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9

filtration to recover the toner particles. As necessary, this procedure may be carried out repeatedly and, after the external additive has been thoroughly separated from the toner particles, the dispersion is dried and the toner particles are collected.

Method for Measuring the Moisture Adsorption/Desorption of the Inorganic Fine Particles

The moisture adsorption/desorption characteristics of the inorganic fine particles are measured using a "BELSORP-aqua3 High Precision Vapor Adsorption Instrument" (Nippon Bel Co., Ltd.). With the "BELSORP-aqua3 High Precision Vapor Adsorption Instrument", a solid-gas equilibrium is achieved under conditions in which only the gas of interest (water for the present disclosure) is present, and the mass of the solid and the vapor pressure are measured at this time.

First, approximately 1 g of the sample is introduced into the sample cell and is degassed at room temperature for 24 hours at 100 Pa or below. After the completion of degassing, the sample weight is exactly weighed followed by setting in the main unit of the instrument and measurement under the following conditions.

air thermostatted chamber temperature: 80.0° C.  
adsorption temperature: 30.0° C.  
adsorbent: H<sub>2</sub>O  
equilibration time: 500 sec  
temperature hold: 60 min  
saturation vapor pressure: 4.245 kPa  
sample tube exhaust rate: normal  
introduction pressure, initial amount of introduction: 0.20  
cm<sup>3</sup> (STP)·g<sup>-1</sup>  
measurement relative pressure P/P<sub>0</sub> (from adsorption process to desorption process is measured): 0.05, 0.10, 0.15, 0.25, 0.35, 0.45, 0.55, 0.65, 0.75, 0.85, 0.90, 0.95, 1.00

The measurement is carried out using these conditions; the moisture adsorption-desorption isotherms are constructed for a temperature of 30.0° C.; and the amount of moisture adsorption Z (mg/g) at a humidity of 100% RH (measurement relative pressure of 1.00) in the adsorption process is calculated.

In addition, the following are also calculated: the value of the amount of moisture adsorption X (mg/g) in the adsorption process at a temperature of 30.0° C. and a relative humidity of 10% RH (measurement relative pressure of 0.10); the value, after the application of a humidity history to a humidity of 100% RH (measurement relative pressure of 1.00), of the amount of moisture adsorption Y (mg/g) in the desorption process at a temperature of 30.0° C. and a relative humidity of 10% RH (measurement relative pressure of 0.10); and their difference, i.e., the value of Y-X.

Method for Measuring the Number-Average Primary Particle Diameter of the Inorganic Fine Particles

The number-average primary particle diameter of the inorganic fine particles is measured using a "JEM-2800" transmission electron microscope (JEOL Ltd.).

Specifically, the toner to be observed is thoroughly dispersed in an epoxy resin, followed by curing for two days in an atmosphere with a temperature of 40° C. to obtain a cured product. Thin-section samples of this cured product are made using an ultrasound ultramicrotome (EM5, Leica), and the long diameter of the primary particles of 100 randomly selected inorganic fine particles is measured using a transmission electron microscope (TEM) in a field of view magnified by a maximum of 50,000 $\times$ . The average value of the measured long diameters is taken to be the number-

average particle diameter. Image Pro PLUS (Nippon Roper K.K.) is used for the measurement.

When the inorganic fine particles as such can be acquired, the number-average particle diameter may be measured by measuring these inorganic fine particles as such using the method described above.

## EXAMPLES

The present disclosure is described in greater detail in the following using examples and comparative examples, but the present disclosure is in no way limited thereto or thereby. The "parts" used in the following formulations are on a mass basis unless specifically indicated otherwise.

## Preparation of Urethane Group-Bearing Monomer

5.0 parts of methanol was introduced into a reactor. This was followed by the dropwise addition of 5.0 parts of Karenz MOI [2-isocyanatoethyl methacrylate] (Showa Denko K. K.) at 40° C. while stirring. After the completion of the dropwise addition, stirring was carried out for 2 hours while maintaining 40° C. The unreacted methanol was then removed using an evaporator to yield a urethane group-bearing monomer.

## Preparation of Urea Group-Bearing Monomer

5.0 parts of dibutylamine was introduced into a reactor. This was followed by the dropwise addition of 5.0 parts of Karenz MOI [2-isocyanatoethyl methacrylate] at room temperature while stirring. Stirring was carried out for 2 hours after the completion of the dropwise addition. The unreacted dibutylamine was then removed using an evaporator to yield a urea group-bearing monomer.

## Preparation of Polymer A0

The following materials were introduced under a nitrogen atmosphere into a reactor fitted with a reflux condenser, stirrer, thermometer, and nitrogen introduction line.

|                                                                                                                                                     |                          |
|-----------------------------------------------------------------------------------------------------------------------------------------------------|--------------------------|
| toluene                                                                                                                                             | 100.0 parts              |
| monomer composition                                                                                                                                 | 100.0 parts              |
| (The monomer composition was provided by mixing the following behenyl acrylate, methacrylonitrile, and styrene in the proportions indicated below.) |                          |
| behenyl acrylate (first polymerizable monomer)                                                                                                      | 67.0 parts (28.88 mol %) |
| methacrylonitrile (second polymerizable monomer)                                                                                                    | 22.0 parts (53.80 mol %) |
| styrene (third polymerizable monomer)                                                                                                               | 11.0 parts (17.33 mol %) |
| t-butyl peroxypivalate<br>(polymerization initiator, Perbutyl PV, NOF Corporation)                                                                  | 0.5 parts                |

While stirring in the aforementioned reactor at 200 rpm, a polymerization reaction was run for 12 hours with heating to 70° C. to obtain a solution in which a polymer of the monomer composition was dissolved in toluene. This solution was then cooled to 25° C. followed by the introduction of the solution while stirring into 1000.0 parts of methanol to precipitate methanol-insoluble matter. The resulting methanol-insoluble matter was filtered off and was additionally washed with methanol, followed by vacuum drying for 24 hours at 40° C. to yield a polymer A0. The polymer A0 had a weight-average molecular weight (Mw) of 68,400, an acid value of 0.0 mg KOH/g, and a melting point of 62° C.

According to the NMR analysis of polymer A0, it contained 28.88 mol % monomer unit derived from behenyl acrylate, 53.80 mol % monomer unit derived from methacrylonitrile, and 17.33 mol % monomer unit derived from styrene.

31

## Preparation of Amorphous Resin

The following starting materials were charged to a heat-dried two-neck flask while introducing nitrogen.

|                                                       |            |
|-------------------------------------------------------|------------|
| polyoxypropylene(2.2)-2,2-bis(4-hydroxyphenyl)propane | 30.0 parts |
| polyoxyethylene(2.2)-2,2-bis(4-hydroxyphenyl)propane  | 33.0 parts |
| terephthalic acid                                     | 21.0 parts |
| dodecylsuccinic acid                                  | 15.0 parts |
| dibutyltin oxide                                      | 0.1 parts  |

After nitrogen replacement within the system using a reduced pressure procedure, stirring was performed for 5 hours at 215° C. This was followed by gradually raising the temperature to 230° C. under reduced pressure while continuing to stir and holding for an additional 2 hours. Once a viscous condition occurred, the reaction was stopped by air cooling to synthesize an amorphous resin that was an amorphous polyester. This amorphous resin had a number-average molecular weight (Mn) of 5,200, a weight-average molecular weight (Mw) of 23,000, and a glass transition temperature (Tg) of 55° C.

## Inorganic Fine Particle B1 Production Example

## Method of Producing Substrate 1

1.0 equivalent, with reference to the iron ion, of a sodium hydroxide solution (contained sodium hexametaphosphate at 1 mass % as P with reference to Fe) was mixed into an aqueous ferrous sulfate solution to prepare an aqueous solution that contained ferrous hydroxide. While maintaining the aqueous solution at pH 9, air was bubbled in and an oxidation reaction was run at 80° C. to prepare a slurry in which seed crystals were produced.

An aqueous ferrous sulfate solution was then added to the slurry so as to provide 1.0 equivalents with reference to the initial amount of alkali (sodium component in the sodium hydroxide). The slurry was held at pH 8 and an oxidation reaction was run while bubbling in air; the pH was adjusted to 6 at the end of the oxidation reaction; and washing with water and drying yielded the substrate 1.

## Method for Treating the Surface of Substrate 1

10,000 parts of the substrate 1 were introduced into a Simpson Mix Muller (Model MSG-0L, SINTOKOGIO, LTD.) and a milling process was carried out for 30 minutes.

This was followed by the introduction into the same machine of 95 parts of n-decytrimethoxysilane as the surface treatment agent, and inorganic fine particle B1 was obtained by operation for 1 hour. The properties of the obtained inorganic fine particle B1 are given in Table 1.

## Inorganic Fine Particle B2 Production Example

## Method of Producing Substrate 2

589.6 parts of methanol, 42.0 parts of water, and 47.1 parts of 28 mass % aqueous ammonia were added with mixing to a 3-L glass reactor equipped with a stirrer, dropping funnels, and a thermometer. The resulting solution was adjusted to 35° C., and, while stirring, the addition of 1100.0 parts of tetramethoxysilane was begun at the same time as the addition of 395.2 parts of 5.4 mass % aqueous ammonia. The tetramethoxysilane was added dropwise over 6 hours and the aqueous ammonia was added dropwise over 5 hours. After completion of the dropwise addition, stirring was continued for an additional 0.5 hours to carry out hydrolysis and yield a methanol-water dispersion of hydrophilic spherical sol-gel silica fine particles.

An ester adapter and a condenser were then mounted on the glass reactor and the dispersion was thoroughly dried at 80° C. under reduced pressure. This step was carried out

32

several tens of times, and the resulting particles were ground using a Pulverizer (Hosokawa Micron Corporation) and processed on a mesh having an aperture of 30 µm to remove coarse particulates and yield a substrate 2.

## 5 Method for Treating the Surface of Substrate 2

A surface treatment was carried out on the substrate 2 using the same method as for the inorganic fine particle B1. The type and amount of the surface treatment agent are given in Table 1. The properties of the obtained inorganic fine particle B2 are given in Table 1.

## Inorganic Fine Particle B3 Production Example

## Method of Producing Substrate 3

Coke and a pulverize of a synthetic rutile were mixed as starting materials; this was introduced into a fluid bed chlorination furnace heated to around a temperature of 1,000° C.; and an exothermic reaction was run with co-fed chlorine gas to obtain a crude titanium tetrachloride. Purification was performed by separating the impurities from the resulting crude titanium tetrachloride to obtain an aqueous titanium tetrachloride solution. While holding this aqueous titanium tetrachloride solution at room temperature, an aqueous sodium hydroxide solution was added to adjust the pH to 7.0 and cause the precipitation of colloidal titanium hydroxide. Ageing was then carried out for 2.5 hours at a temperature of 62° C. to provide a slurry of titanium oxide base particles having a rutile nucleus. This was followed by filtration and washing; the resulting wet cake was heat treated for 24 hours at 120° C.; and milling was performed followed by processing on a mesh having an aperture of 50 µm to remove coarse particulates and yield a substrate 3.

## Method for Treating the Surface of Substrate 3

A surface treatment was carried out using the same method as for the inorganic fine particle B1. The type and amount of the surface treatment agent are given in Table 1. The properties of the obtained inorganic fine particle B3 are given in Table 1.

## Inorganic Fine Particle B4 Production Example

## Method of Producing Substrate 4

40 Aluminum hydroxide was introduced into a stainless steel autoclave, and the temperature was raised to 1500° C. with the autoclave sealed and this temperature was held for 3 hours. The resulting particles were ground with a ball mill and processed on a mesh with an aperture of 50 µm to remove the coarse particulates and provide substrate 4.

## Method for Treating the Surface of Substrate 4

A surface treatment was carried out using the same method as for the inorganic fine particle B1. The type and amount of the surface treatment agent are given in Table 1.

50 The properties of the obtained inorganic fine particle B4 are given in Table 1.

## Inorganic Fine Particle B5 Production Example

## Method of Producing Substrate 5

9.5 L of an aqueous suspension (10%) of slaked lime (calcium hydroxide:  $\text{Ca}(\text{OH})_2$ ) was introduced into a 45-L pressure apparatus and calcium carbonate particles were synthesized by bubbling with carbon dioxide gas. 25° C. was used for the reaction temperature and 100%-pure carbon dioxide gas (bubbling rate: 10 L/min) was used for the carbon dioxide gas, and the reaction was stopped at the stage at which the pH of the reaction solution reached 7. The resulting slurry was processed on a mesh with an aperture of 50 µm to remove the coarse particulates and was dried to provide substrate 5.

## 65 Method for Treating the Surface of Substrate 5

A surface treatment was carried out using the same method as for the inorganic fine particle B1. The type and

amount of the surface treatment agent are given in Table 1. The properties of the obtained inorganic fine particle B5 are given in Table 1.

Inorganic Fine Particles B6 to B8 and B10 Production Example

A surface treatment was carried out on the substrate 1 using the same method as for the inorganic fine particle B1. The type and amount of the surface treatment agent are given in Table 1. The properties of the obtained inorganic fine particles B6 to B8 and B10 are given in Table 1.

Inorganic Fine Particle B9 Production Example

The substrate 1 was used the inorganic fine particle B9. The properties are given in Table 1.

Inorganic Fine Particle B11 Production Example

The surface treatment agent indicated in Table 1 was diluted with 200 parts of toluene to give a solids fraction of 10 mass %. This was thoroughly mixed to prepare a coating resin solution.

100 parts of the substrate 1 was added to 32 parts of the coating resin solution and nitrogen was introduced while reducing the pressure and heating to a temperature of 65° C. was carried out, and stirring was performed using a universal mixer agitator (Fuji Paudal Co., Ltd.). While stirring, the coating resin solution was introduced in five additions (6.4 parts per addition) and the solvent was removed. After cooling to room temperature, the resulting surface-treated inorganic fine particles were transferred to a *Julia Mixer* (Tokuju Corporation) and were heat treated for 2 hours at 160° C. under a nitrogen atmosphere. The coarse particulates were removed by processing on a mesh with an aperture of 50 µm to provide inorganic fine particle B11. The properties of the resulting inorganic fine particle B11 are shown in Table 1.

Toner 1 Production Example

Toner Production by Suspension Polymerization

Toner Particle 1 Production

850 mass parts of an aqueous 0.1 mol/L Na<sub>3</sub>PO<sub>4</sub> solution was added to a vessel equipped with a ClearMix high-speed stirrer (M Technique Co., Ltd.), and the temperature was raised to 60° C. while stirring at a rotational peripheral velocity of 33 m/s. To this was added 68 mass parts of an aqueous 1.0 mol/L CaCl<sub>2</sub> solution to prepare an aqueous medium that contained the microtine sparingly water-soluble dispersing agent Ca<sub>3</sub>(PO<sub>4</sub>)<sub>2</sub>.

A solution was also prepared by mixing and dissolving the following materials using a propeller stirrer. The constitution and properties of the inorganic fine particles that were used are given in Table 1. A stirrer rotation rate of 100 r/min was used in the mixing of these materials. The mixture was prepared from the following:

|                                                                                                                                                                            |                          |
|----------------------------------------------------------------------------------------------------------------------------------------------------------------------------|--------------------------|
| monomer composition<br>(The monomer composition was provided by mixing the following behenyl acrylate, methacrylonitrile, and styrene in the proportions indicated below.) | 100.0 parts              |
| behenyl acrylate (first polymerizable monomer)                                                                                                                             | 67.0 parts (28.88 mol %) |
| methacrylonitrile (second polymerizable monomer)                                                                                                                           | 22.0 parts (53.80 mol %) |
| styrene (third polymerizable monomer)                                                                                                                                      | 11.0 parts (17.33 mol %) |
| inorganic fine particle B1                                                                                                                                                 | 65.0 parts               |
| charge control agent (aluminum di-t-butylsalicylate)                                                                                                                       | 0.7 parts                |
| release agent<br>(product name: HNP-51, melting point = 78° C., Nippon Seiro Co., Ltd.)                                                                                    | 10.0 parts               |
| toluene                                                                                                                                                                    | 100.0 parts              |

This mixture was introduced into an attritor (Nippon Coke & Engineering Co., Ltd.), and a starting material dispersion was obtained by dispersing for 2 hours at 200 rpm using zirconia beads with a diameter of 5 mm.

5 Otherwise, 735.0 parts of deionized water and 16.0 parts of trisodium phosphate (dodecahydrate) were added to a vessel outfitted with a Homomixer high-speed stirrer (PRI-MIX Corporation) and a thermometer, and the temperature was raised to 60° C. while stirring at 12,000 rpm. To this was 10 added an aqueous calcium chloride solution of 9.0 parts calcium chloride (dihydrate) dissolved in 65.0 parts of deionized water, and stirring was carried out for 30 minutes at 12,000 rpm while maintaining 60° C. To this was added 15 10% hydrochloric acid to adjust the pH to 6.0 and obtain an aqueous medium that contained a dispersion stabilizer.

The starting material dispersion was transferred to a vessel outfitted with a stirrer and thermometer, and the temperature was raised to 60° C. while stirring at 100 rpm. To this was added 8.0 parts of the polymerization initiator 20 t-butyl peroxypropionate (Perbutyl PV, NOF Corporation); stirring was performed for 5 minutes at 100 rpm while holding at 60° C.; and this was introduced into the aqueous medium that was being stirred at 12,000 rpm with the high-speed stirrer. A granulation solution was obtained by 25 continuing to stir for 20 minutes at 12,000 rpm with the high-speed stirrer while holding at 60° C.

The granulation solution was transferred to a reactor outfitted with a reflux condenser, stirrer, thermometer, and nitrogen introduction line, and the temperature was raised to 30 70° C. while stirring at 150 rpm under a nitrogen atmosphere. A polymerization reaction was run for 10 hours at 150 rpm while holding at 70° C. This was followed by removal of the reflux condenser from the reactor; raising the temperature of the reaction solution to 95° C.; and removing 35 the toluene by stirring for 5 hours at 150 rpm while holding at 95° C. to yield a toner particle dispersion.

The resulting toner particle dispersion was cooled to 20° C. while stirring at 150 rpm, and, while maintaining this stirring in this condition, dilute hydrochloric acid was then 40 added to bring the pH to 1.5 and dissolve the dispersion stabilizer. The solid fraction was filtered off and thoroughly washed with deionized water, followed by vacuum drying for 24 hours at 40° C. to obtain a toner particle 1 containing a polymer A1 of the monomer composition.

45 In addition, a polymer A1' was obtained proceeding entirely as in the Toner Particle 1 Production method, but without using the inorganic fine particles, charge control agent, and release agent.

The polymer A1' had a weight-average molecular weight 50 (M<sub>w</sub>) of 56,000 and had a melting point of 62° C.

According to the NMR analysis of polymer A1', it contained 28.88 mol % monomer unit derived from behenyl acrylate, 53.80 mol % monomer unit derived from methacrylonitrile, and 17.33 mol % monomer unit derived from 55 styrene.

The polymer A1 and polymer A1' were assumed to have the same properties because they were produced in the same manner.

Toner 1 Preparation

60 0.5 parts of a hydrophobed colloidal silica (product name: R-202, Degussa) was added to 100 parts of the obtained toner particle 1 and a toner 1 was prepared by mixing using a Henschel mixer.

Toners 2 to 24, 29 to 36, 43 to 45, 49, and 50 Production 65 Example

Toner particles 2 to 24, 29 to 36, 43 to 45, 49, and 50 were obtained proceeding entirely as in the Toner 1 Production

## 35

Example, but changing the type and number of parts of addition of the polymerizable monomer and inorganic fine particles used as indicated in Table 2.

External addition was also carried out as in the Toner 1 Production Example to obtain toners 2 to 24, 29 to 36, 43 to 45, 49, and 50. The properties of toners 2 to 24, 29 to 36, 43 to 45, 49, and 50 are given in Table 3.

## Toners 25 to 28 and 46 Production Example

Toner particles 25 to 28 and 46 were obtained proceeding entirely as in the Toner 1 Production Example, but adding 6.5 parts of carbon black during mixing and dissolution of the materials using the propeller stirrer.

External addition was also carried out as in the Toner 1 Production Example to obtain toners 25 to 28 and 46. The properties of toners 25 to 28 and 46 are given in Table 3.

## Toner 37 Production Example

[Production of Toner by Emulsion Aggregation]  
(Preparation of a Polymer Dispersion)

|            |             |
|------------|-------------|
| toluene    | 300.0 parts |
| polymer A0 | 100.0 parts |

These materials were weighed out and mixed and dissolution was carried out at 90° C.

Separately, 5.0 parts of sodium dodecylbenzenesulfonate and 10.0 parts of sodium laurate were added to 700.0 parts of deionized water and dissolution was performed with heating at 90° C. The aforementioned toluene solution and the aqueous solution were then mixed and stirring was carried out at 7,000 rpm using a T. K. Robomix ultrahigh-speed stirrer (PRIMIX Corporation). Emulsification was also performed at a pressure of 200 MPa using a Nanomizer high-pressure impact-type disperser (Yoshida Kikai Co., Ltd.). This was followed by removal of the toluene using an evaporator and adjustment of the concentration with deionized water to obtain a polymer dispersion having a polymer fine particle concentration of 20%.

The 50% particle diameter (D50) on a volume basis of the polymer fine particles was measured at 0.40 µm using a Nanotrac UPA-EX150 dynamic light-scattering particle size distribution analyzer (Nikkiso Co., Ltd.).

## Preparation of Release Agent Dispersion 1

|                                                                           |             |
|---------------------------------------------------------------------------|-------------|
| release agent<br>(HNP-51, melting point = 78° C., Nippon Seiro Co., Ltd.) | 100.0 parts |
| Neogen RK anionic surfactant (Dai-ichi Kogyo Seiyaku Co., Ltd.)           | 5.0 parts   |
| deionized water                                                           | 395.0 parts |

The preceding materials were weighed and introduced into a mixing container equipped with a stirrer and were heated to 90° C., and a dispersion treatment was then carried out for 60 minutes by circulation to a ClearMix W-Motion (M Technique Co., Ltd.). The following dispersion conditions were used.

rotor outer diameter=3 cm

clearance=0.3 mm

rotor rotation rate=19,000 r/min

screen rotation rate=19,000 r/min

After the dispersion treatment, cooling to 40° C. was carried out using cooling process conditions of a rotor rotation rate of 1,000 r/min, a screen rotation rate of 0 r/min, and a cooling rate of 10° C./min, to obtain a release agent dispersion 1 having a 20% concentration of release agent fine particle 1.

## 36

The 50% particle diameter (D50) on a volume basis of release agent fine particle 1 was measured at 0.15 µm using a Nanotrac UPA-EX150 dynamic light-scattering particle size distribution analyzer (Nikkiso Co., Ltd.).

## Preparation of an Inorganic Fine Particle Dispersion

|                                                                                               |                         |
|-----------------------------------------------------------------------------------------------|-------------------------|
| inorganic fine particle B1<br>Neogen RK anionic surfactant (Dai-ichi Kogyo Seiyaku Co., Ltd.) | 50.0 parts<br>7.5 parts |
| deionized water                                                                               | 442.5 parts             |

These materials were weighed out and mixed and dispersion was performed for approximately 1 hour using a Nanomizer high-pressure impact-type disperser (Yoshida Kikai Co., Ltd.) to obtain an inorganic fine particle dispersion 1 having an inorganic fine particle concentration of 10 mass %.

## Toner 37 Production

|                                                                                                             |                                                         |
|-------------------------------------------------------------------------------------------------------------|---------------------------------------------------------|
| polymer dispersion<br>release agent dispersion 1<br>inorganic fine particle dispersion 1<br>deionized water | 500.0 parts<br>50.0 parts<br>650.0 parts<br>160.0 parts |
|-------------------------------------------------------------------------------------------------------------|---------------------------------------------------------|

These materials were introduced into a round stainless steel flask and were mixed. Dispersion was then carried out for 10 minutes at 5,000 r/min using an Ultra-Turrax T50 homogenizer (IKA). The pH was adjusted to 3.0 by adding a 1.0% aqueous nitric acid solution; then, using a stirring blade and a heating water bath, heating to 58° C. was carried out while adjusting the rotation rate as appropriate so as to stir the mixture. The volume-average particle diameter of the aggregated particles that formed was monitored as appropriate using a Coulter Multisizer III, and, at the point at which 6.0 µm aggregated particles had been formed, the pH was brought to 9.0 using a 5% aqueous sodium hydroxide solution. Stirring was then continued while heating to 75° C. The aggregated particles were fused by holding for 1 hour at 75° C.

Polymer crystallization was then promoted by cooling to 50° C. and holding for 3 hours.

This was followed by cooling to 25° C., filtration and solid-liquid separation, and then washing with deionized water. After the completion of washing, drying using a vacuum dryer yielded a toner particle 37 having a weight-average particle diameter (D4) of 6.07 µm.

Toner 37 was obtained by carrying out external addition as described in the Toner 1 Production Example on the toner particle 37. The properties of the toner 37 are given in Table 3.

## Toner 38 Production Example

## Toner Production by Dissolution Suspension

## 55 Fine Particle Dispersion 1 Preparation

683.0 parts of water, 11.0 parts of sodium methacrylic acid/ethylene oxide (EO) adduct sulfate (Eleminol RS-30, Sanyo Chemical Industries, Ltd.), 130.0 parts of styrene, 138.0 parts of methacrylic acid, 184.0 parts of n-butyl acrylate, and 1.0 parts of ammonium persulfate were introduced into a reactor fitted with a stirring rod and a thermometer, and a white suspension was obtained upon stirring for 15 minutes at 400 rpm. Heating was carried out and the temperature in the system was raised to 75° C. and a reaction was carried out for 5 hours.

An additional 30.0 parts of a 1% aqueous ammonium persulfate solution was added and a fine particle dispersion

37

1 of a vinyl polymer was obtained by ageing for 5 hours at 75° C. The 50% particle diameter (D50) on a volume basis of fine particle dispersion 1 was measured at 0.15  $\mu$ m using a Nanotrac UPA-EX150 dynamic light-scattering particle size distribution analyzer (Nikkiso Co., Ltd.).

#### Preparation of an Inorganic Fine Particle Dispersion 2

|                            |             |
|----------------------------|-------------|
| inorganic fine particle B1 | 100.0 parts |
| ethyl acetate              | 150.0 parts |
| glass beads (1 mm)         | 200.0 parts |

These materials were introduced into a heat-resistant glass vessel; dispersion was performed for 5 hours using a paint shaker; and the glass beads were removed using a nylon mesh to yield an inorganic fine particle dispersion 2. The 50% particle diameter (D50) on a volume basis of the inorganic fine particle dispersion was measured at 0.20  $\mu$ m using a Nanotrac UPA-EX150 dynamic light-scattering particle size distribution analyzer (Nikkiso Co., Ltd.).

#### Preparation of Release Agent Dispersion 2

|                                                                              |            |
|------------------------------------------------------------------------------|------------|
| release agent<br>(HNP-51, melting point = 78° C.,<br>Nippon Seiro Co., Ltd.) | 20.0 parts |
| ethyl acetate                                                                | 80.0 parts |

The preceding were introduced into a sealable reactor and were stirred and heated at 80° C. Then, while gently stirring the system at 50 rpm, cooling to 25° C. was performed over 3 hours to yield a milky white liquid.

This solution was introduced into a heat-resistant vessel together with 30.0 parts of glass beads having a diameter of 1 mm; dispersion was carried out for 3 hours using a paint shaker (Toyo Seiki Seisaku-sho Ltd.); and the glass beads were removed using a nylon mesh to yield a release agent dispersion 2. The 50% particle diameter (D50) on a volume basis of release agent dispersion 2 was measured at 0.23  $\mu$ m using a Nanotrac UPA-EX150 dynamic light-scattering particle size distribution analyzer (Nikkiso Co., Ltd.).

#### Preparation of Oil Phase

|               |             |
|---------------|-------------|
| polymer A0    | 100.0 parts |
| ethyl acetate | 85.0 parts  |

These materials were introduced into a beaker and stirring was carried out for 1 minute at 3,000 rpm using a Disper (Tokushu Kika Kogyo Co., Ltd.).

release agent dispersion 2 (20% solids) 50.0 parts  
inorganic fine particle dispersion 2 (40% solids) 162.5  
parts  
ethyl acetate 5.0 parts

These materials were introduced into a beaker and an oil phase was prepared by stirring for 3 minutes at 6,000 rpm using a Disper (Tokushu Kika Kogyo Co., Ltd.).

#### Preparation of Aqueous Phase

|                                                                 |             |
|-----------------------------------------------------------------|-------------|
| fine particle dispersion 1                                      | 15.0 parts  |
| aqueous solution of sodium dodecyldiphenyl<br>ether disulfonate | 30.0 parts  |
| (Eleminol MON7, Sanyo Chemical Industries,<br>Ltd.)             |             |
| deionized water                                                 | 955.0 parts |

38

These materials were introduced into a beaker and an aqueous phase was prepared by stirring for 3 minutes at 3,000 rpm using a Disper (Tokushu Kika Kogyo Co., Ltd.).

#### Toner 38 Production

5 The oil phase was introduced into the aqueous phase and dispersion was carried out for 10 minutes at a rotation rate of 10,000 rpm using a T. K. Homomixer (Tokushu Kika Kogyo Co., Ltd.). This was followed by solvent removal for 30 minutes at 30° C. under a reduced pressure of 50 mmHg. 10 Filtration was then performed, and the process of filtration and redispersion in deionized water was repeated until the conductivity of the slurry reached 100  $\mu$ S to remove the surfactant and yield a filter cake.

15 This filter cake was vacuum dried followed by air classification to obtain a toner particle 38.

Toner 38 was obtained by carrying out external addition as described in the Toner 1 Production Example on the toner particle 38. The properties of the toner 38 are given in Table 20 3.

#### Toner 39 Production Example

#### Production of Toner by Pulverization

|                                                                              |             |
|------------------------------------------------------------------------------|-------------|
| polymer A0                                                                   | 100.0 parts |
| inorganic fine particle B1                                                   | 65.0 parts  |
| release agent<br>(HNP-51, melting point = 78° C.,<br>Nippon Seiro Co., Ltd.) | 2.0 parts   |
| charge control agent (T-77, Hodogaya<br>Chemical Co., Ltd.)                  | 2.0 parts   |
|                                                                              |             |

These materials were pre-mixed using an FM mixer (Nippon Coke & Engineering Co., Ltd.) followed by melt-kneading with a twin-screw kneading extruder (Model 35 PCM-30, Ikegai Ironworks Corporation).

35 The resulting kneaded material was cooled and coarsely pulverized using a hammer mill and was then pulverized using a mechanical pulverizer (T-250, Turbo Kogyo Co., Ltd.). The resulting finely pulverized powder was classified 40 using a Coanda effect-based multi-grade classifier to yield a toner particle 39 having a weight-average particle diameter (D4) of 7.0  $\mu$ m.

Toner 39 was obtained by carrying out external addition 45 as described in the Toner 1 Production Example on the toner particle 39. The properties of the toner 39 are given in Table 2.

#### Toners 40 to 42 Production Example

#### Preparation of an Amorphous Resin Dispersion

|                 |             |
|-----------------|-------------|
| toluene         | 300.0 parts |
| amorphous resin | 100.0 parts |

55 These materials were weighed out and mixed and dissolution was carried out at 90° C.

Separately, 5.0 parts of sodium dodecylbenzenesulfonate and 10.0 parts of sodium laurate were added to 700.0 parts of deionized water and dissolution was carried out with 60 heating at 90° C.

The toluene solution was then mixed with the aqueous solution and stirring at 7,000 rpm was performed using a T. K. Robomix ultrahigh-speed stirrer (PRIMIX Corporation).

Emulsification was performed at a pressure of 200 MPa 65 using a Nanomizer high-pressure impact-type disperser (Yoshida Kikai Co., Ltd.). The toluene was subsequently removed using an evaporator and the concentration was

39

adjusted using deionized water to yield an amorphous resin dispersion having a 20% concentration of amorphous resin fine particles.

The 50% particle diameter (D50) on a volume basis of the amorphous resin fine particles was measured at 0.38  $\mu\text{m}$  using a Nanotrac UPA-EX150 dynamic light-scattering particle size distribution analyzer (Nikkiso Co., Ltd.).

#### Production of Toners 40 to 42

Toner particles 40 to 42 were obtained proceeding entirely as in the Toner 37 Production Example, but changing the amount of use of the dispersions as indicated in Table 5.

Toners 40 to 42 were obtained by carrying out external addition as described in the Toner 37 Production Example on the toner particles 40 to 42. The properties of the toners 40 to 42 are given in Table 3.

#### Toners 47 and 48 Production Example

Toner particles 47 and 48 were obtained proceeding entirely as in the Toner 39 Production Example, but changing the type and number of parts of addition of the polymerizable monomer and inorganic fine particles used as indicated in Table 2.

External addition was also carried out as in the Toner 1 Production Example to obtain toners 47 and 48. The properties of toners 47 and 48 are given in Table 3.

#### Example 1

The following evaluations were performed on toner 1.

##### 1 Evaluation of the Low-Temperature Fixability

Using a LaserJet Pro 400 M451 from HP that had been modified to enable operation with the fixing unit detached, an unfixed image with an image pattern in which 10 mm  $\times$  10 mm square images were uniformly arrayed at 9 points over the entire transfer paper was output.

Fox River Bond (A4, 90 g/m<sup>2</sup>) was used as the transfer paper, and 0.70 mg/cm<sup>2</sup> was used for the toner laid-on level on the transfer paper. The toner was held for 48 hours in a normal-temperature, normal-humidity (N/N) environment (23° C., 60% RH) prior to paper feed.

For the fixing unit, the fixing unit of a LaserJet P2055 from HP was removed therefrom and was used as an external fixing unit that was set up to also operate outside the laser beam printer.

The aforementioned unfixed image was fed using a process speed of 210 mm/sec with the fixation temperature at the external fixing unit being raised in 10° C. steps from a temperature of 100° C.

After passage through the external fixing unit, the fixed image was rubbed with lens cleaning paper ("Dusper®" (Ozu Paper Co., Ltd.)) under a load of 50 g/cm<sup>2</sup>. The fixing onset temperature was taken to be the temperature at which the percentage decline in density pre-versus-post-rubbing was equal to or less than 20%, and the low-temperature fixability was evaluated using the following criteria.

The results of the evaluation are given in Table 6.

##### Evaluation Criteria

- A: the fixing onset temperature is 100° C.
- B: the fixing onset temperature is 110° C.
- C: the fixing onset temperature is 120° C.
- D: the fixing onset temperature is equal to or greater than 130° C.

##### 2 Evaluation of the Heat-Resistant Storability

The heat-resistant storability was evaluated in order to evaluate the stability during storage.

Approximately 5 g of toner 1 was introduced into a 100-mL polypropylene cup; this was held for 10 days in an environment with a temperature of 50° C. and a humidity of

40

20%; and the degree of toner aggregation was measured as described below and was evaluated using the criteria given below.

The following was used as the measurement instrumentation: a "Model 1332A Digital Vibration Meter" (Showa Sokki Co., Ltd.) digital display vibration meter connected to the side surface of the vibrating platform of a "Powder Tester" (Hosokawa Micron Corporation).

The following were stacked, in sequence from the bottom, on the vibrating platform of the Powder Tester: a sieve with an aperture of 38  $\mu\text{m}$  (400 mesh), a sieve with an aperture of 75  $\mu\text{m}$  (200 mesh), and a sieve with an aperture of 150  $\mu\text{m}$  (100 mesh). The measurement was performed as follows in a 23° C./60% RH environment.

(1) The vibration amplitude of the vibrating platform was preliminarily adjusted so as to provide 0.60 mm (peak-to-peak) for the value of the displacement on the digital display vibration meter.

(2) The toner, after its standing for 10 days as described above, was preliminarily held for 24 hours in a 23° C./60% RH environment. 5 g of the toner was then exactly weighed out and was gently loaded on the sieve having an aperture of 150  $\mu\text{m}$ , which was in the uppermost position.

(3) The screens were vibrated for 15 seconds; the mass of toner retained on each sieve was then measured; and the degree of aggregation was calculated based on the following formula. The results of the evaluation are given in Table 6.

$$\text{degree of aggregation}(\%) = \frac{\{( \text{sample mass (g)} \text{ on the sieve with an aperture of } 150 \mu\text{m}) / 5 \text{ (g)}\} \times 100 + \{( \text{sample mass (g)} \text{ on the sieve with an aperture of } 75 \mu\text{m}) / 5 \text{ (g)}\} \times 100 \times 0.6 + \{( \text{sample mass (g)} \text{ on the sieve with an aperture of } 38 \mu\text{m}) / 5 \text{ (g)}\} \times 100 \times 0.2}{100 \times 0.2}$$

The evaluation criteria are as follows.

- A: the degree of aggregation is less than 20%
- B: the degree of aggregation is at least 20%, but less than 25%
- C: the degree of aggregation is at least 25%, but less than 30%
- D: the degree of aggregation is equal to or greater than 30%

##### 3 Evaluation of the Durability

The toner 1 obtained as described above was loaded into a LaserJet Pro 400 M451 from HP, after which the print paper was also loaded.

Fox River Bond (A4, 90 g/m<sup>2</sup>) was used for the transfer paper.

An image with a print percentage of 1% was continuously output in a 23° C./60% RH environment.

After the output of each 500 prints, a solid image and a halftone image were output, and the presence/absence of the production of vertical streaks originating with toner fusion to the control member, i.e., the production of development streaks, was visually inspected.

10,500 prints were ultimately output. The results of the evaluation are given in Table 6.

## [Evaluation Criteria]

- A: no vertical streaks even at 10,500 prints  
 B: vertical streaks occur at more than 9,000 prints, but not more than 10,500 prints  
 C: vertical streaks occur at more than 7,500 prints, but not more than 9,000 prints  
 D: vertical streaks occur at not more than 7,500 prints

## 4 Evaluation of the Discharged Paper Adhesion Behavior

The toner 1 obtained as described above was loaded into a LaserJet Pro 400 M451 from HP, after which the print paper was also loaded.

Fox River Bond (A4, 90 g/m<sup>2</sup>) was used for the transfer paper. Prior to paper feed, the toner has held for 24 hours in a high-temperature, high-humidity (H/H) environment (32.5° C., 80% RH).

Using a test chart with a print percentage of 12%, a duplex 10-sheet continuous print test was carried out in the H/H environment. Then, with the 10 sheets stacked, a load was applied for 1 hour by stacking with 7 reams (corresponded to 3,500 sheets) of the unopened transfer paper (500 sheets/ream), and the condition upon unstacking was evaluated. The results of the evaluation are given in Table 6.

- A: Discharged sheet adhesion is not produced.  
 B: While sticking between sheets is seen, image defects after unstacking are not seen.  
 C: Minor image defects are seen after unstacking.  
 D: Significant image defects are seen after unstacking.

## 5 Fogging in a High-Temperature, High-Humidity Environment

The toner 1 obtained as described above was loaded into a LaserJet Pro 400 M451 from HP, after which the print paper was also loaded.

Fox River Bond (A4, 90 g/m<sup>2</sup>) was used for the transfer paper. In addition, prior to paper feed, the toner has held for 3 days in a high-temperature, high-humidity (H/H) environment (32.5° C., 80% RH).

While operating in the H/H environment, a single print of an image having a white background region was printed out.

The reflectance was measured on the obtained image using a reflection densitometer (Reflectometer Model TC-6DS, Tokyo Denshoku Co., Ltd.). A green filter was used for the filter used for the measurement. The evaluation was performed using the following criteria and using Ds (%) for the poorest value of the reflectance in the white background region, Dr (%) for the reflectance of the transfer paper prior to image formation, and Dr-Ds for the fogging. The results of the evaluation are given in Table 6.

- A: the fogging is less than 1.0%  
 B: the fogging is at least 1.0%, but less than 3.0%  
 C: the fogging is at least 3.0%, but less than 5.0%  
 D: the fogging is equal to or greater than 5.0%

## 6 Ghosting in a Low-Temperature, Low-Humidity Environment

The toner 1 obtained as described above was loaded into a LaserJet Pro 400 M451 from HP, after which the print paper was also loaded.

Fox River Bond (A4, 90 g/m<sup>2</sup>) was used for the transfer paper. In addition, prior to paper feed, the toner has held for 3 days in a low-temperature, low-humidity (L/L) environment (15° C., 10% RH).

A ghosting evaluation image was output after 300 prints of a solid white image had been printed out in the L/L environment.

For the ghosting evaluation image, seven 15 mm×15 mm solid images were lined up in one row widthwise using a 15 mm gap at a position 5 mm from the upper edge of the transfer paper and a halftone image with a toner laid on level of 0.20 mg/cm<sup>2</sup> was placed below the solid image.

The following formula was used to calculate the difference in the reflection density, measured using a MacBeth reflection densitometer, in the halftone region of this image between the location (black print area) where the solid black image was formed at the first rotation of the developing roller and the location (nonimage area) where it was not.

$$\text{“reflection density difference”} = (\text{reflection density of the image for the region which was the nonimage area in the first rotation of the developing roller}) - (\text{reflection density of the image for the region which was the black print area in the first rotation of the developing roller})$$

A smaller reflection density difference is regarded as being indicative of less ghosting in this evaluation. This reflection density difference was evaluated used the following criteria. The results of the evaluation are given in Table 6.

- A: equal to or greater than 0.00, but less than 0.03  
 B: equal to or greater than 0.03, but less than 0.06  
 C: equal to or greater than 0.06, but less than 0.10  
 D: equal to or greater than 0.10, but less than 0.15  
 E: equal to or greater than 0.15

## Examples 2 to 45

The same evaluations as for toner 1 were carried out on toners 2 to 45. The results are given in Table 6.

## Comparative Examples 1 to 5

The same evaluations as for toner 1 were carried out on toners 46 to 50. The results are given in Table 6.

The abbreviations used in the tables expand as follows.

- BEA: behenyl acrylate  
 BEMA: behenyl methacrylate  
 SA: stearyl acrylate  
 MYA: myricyl acrylate  
 OA: octacosyl acrylate  
 HA: hexadecyl acrylate  
 MN: methacrylonitrile  
 AN: acrylonitrile  
 HPMA: 2-hydroxypropyl methacrylate  
 AM: acrylamide  
 UT: urethane group-bearing monomer  
 UR: urea group-bearing monomer  
 AA: acrylic acid  
 VA: vinyl acetate  
 MA: methyl acrylate  
 St: styrene  
 MM: methyl methacrylate

TABLE 1

| Surface-treated inorganic fine particle |                  |                                                                      |                                  |          |            |                                       |      |
|-----------------------------------------|------------------|----------------------------------------------------------------------|----------------------------------|----------|------------|---------------------------------------|------|
| Inorganic fine particle                 |                  | Type of treatment agent                                              | Amount of use of treatment agent |          |            | Number-average particle diameter (μm) |      |
| No.                                     | Substrate        |                                                                      | (parts)                          | Z (mg/g) | Y-X (mg/g) | *1                                    |      |
| B1                                      | Magnetite        | n-C <sub>10</sub> H <sub>21</sub> Si(CH <sub>3</sub> O) <sub>3</sub> | 95                               | 3.0      | 0.30       | 0.21                                  | 0.94 |
| B2                                      | SiO <sub>2</sub> | n-C <sub>10</sub> H <sub>21</sub> Si(CH <sub>3</sub> O) <sub>3</sub> | 88                               | 2.8      | 0.29       | 0.08                                  | 0.87 |

TABLE 1-continued

| Surface-treated inorganic fine particle |                                |                                                                      |                                          |            |                                       |      |      |
|-----------------------------------------|--------------------------------|----------------------------------------------------------------------|------------------------------------------|------------|---------------------------------------|------|------|
| Inorganic fine particle No.             | Substrate                      | Type of treatment agent                                              | Amount of use of treatment agent (parts) |            | Number-average particle diameter (μm) |      |      |
|                                         |                                |                                                                      | Z (mg/g)                                 | Y-X (mg/g) | Y-X                                   | Y-X  | *1   |
| B3                                      | TiO <sub>2</sub>               | n-C <sub>10</sub> H <sub>21</sub> Si(CH <sub>3</sub> O) <sub>3</sub> | 90                                       | 3.4        | 0.31                                  | 0.12 | 0.89 |
| B4                                      | Al <sub>2</sub> O <sub>3</sub> | n-C <sub>2</sub> H <sub>5</sub> Si(CH <sub>3</sub> O) <sub>3</sub>   | 235                                      | 4.8        | 0.33                                  | 0.15 | 2.30 |
| B5                                      | Calcium carbonate              | n-C <sub>10</sub> H <sub>21</sub> Si(CH <sub>3</sub> O) <sub>3</sub> | 111                                      | 5.5        | 0.32                                  | 0.50 | 1.10 |
| B6                                      | Magnetite                      | n-C <sub>4</sub> H <sub>9</sub> Si(CH <sub>3</sub> O) <sub>3</sub>   | 204                                      | 1.5        | 0.12                                  | 0.21 | 2.00 |
| B7                                      | Magnetite                      | n-C <sub>16</sub> H <sub>33</sub> Si(CH <sub>3</sub> O) <sub>3</sub> | 30                                       | 10.0       | 0.25                                  | 0.21 | 0.30 |
| B8                                      | Magnetite                      | n-C <sub>10</sub> H <sub>21</sub> Ti(CH <sub>3</sub> O) <sub>3</sub> | 152                                      | 1.6        | 0.07                                  | 0.21 | 1.50 |
| B9                                      | Magnetite                      | —                                                                    | —                                        | 14.0       | 0.39                                  | 0.21 | —    |
| B10                                     | Magnetite                      | n-C <sub>10</sub> H <sub>21</sub> Si(CH <sub>3</sub> O) <sub>3</sub> | 113                                      | 1.1        | 0.05                                  | 0.21 | 1.12 |
| B11                                     | Magnetite                      | n-CH <sub>2</sub> =CHCOOC <sub>16</sub> H <sub>33</sub>              | 320                                      | 12.0       | 0.26                                  | 0.21 | 3.10 |

\*1: Amount of carbon (mass %) contained by the inorganic fine particles, with reference to the inorganic fine particles.

TABLE 2

TABLE 2-continued

| Polymer A |                         |      |                             |      |                              |      |                             | 20   | Polymer A |                         |       |                             |      |                              |      |                             |      |
|-----------|-------------------------|------|-----------------------------|------|------------------------------|------|-----------------------------|------|-----------|-------------------------|-------|-----------------------------|------|------------------------------|------|-----------------------------|------|
| Toner     | Inorganic fine particle |      | First polymerizable monomer |      | Second polymerizable monomer |      | Third polymerizable monomer |      | Toner     | Inorganic fine particle |       | First polymerizable monomer |      | Second polymerizable monomer |      | Third polymerizable monomer |      |
|           | No.                     | Type | parts                       | Type | parts                        | Type | parts                       | Type | parts     | No.                     | Type  | parts                       | Type | parts                        | Type | parts                       |      |
| 1         | B1                      | 65.0 | BEA                         | 67.0 | MN                           | 22.0 | St                          | 11.0 | 27        | B4                      | 65.0  | BEA                         | 65.0 | MN                           | 6.0  | St                          | 29.0 |
| 2         | B1                      | 65.0 | BEA                         | 67.0 | AN                           | 22.0 | St                          | 11.0 | 28        | B5                      | 65.0  | BEA                         | 65.0 | MN                           | 6.0  | St                          | 29.0 |
| 3         | B1                      | 65.0 | BEA                         | 50.0 | HPMA                         | 40.0 | St                          | 10.0 | 29        | B6                      | 65.0  | BEA                         | 65.0 | MN                           | 6.0  | St                          | 29.0 |
| 4         | B1                      | 65.0 | BEA                         | 60.0 | VA                           | 30.0 | St                          | 10.0 | 30        | B7                      | 65.0  | BEA                         | 65.0 | MN                           | 6.0  | St                          | 29.0 |
| 5         | B1                      | 65.0 | BEA                         | 60.0 | MA                           | 30.0 | St                          | 10.0 | 31        | B8                      | 65.0  | BEA                         | 65.0 | MN                           | 6.0  | St                          | 29.0 |
| 6         | B1                      | 65.0 | BEA                         | 65.0 | AM                           | 25.0 | St                          | 10.0 | 32        | B10                     | 65.0  | BEA                         | 65.0 | MN                           | 6.0  | St                          | 29.0 |
| 7         | B1                      | 65.0 | BEA                         | 61.0 | AA                           | 9.0  | MM                          | 30.0 | 33        | B1                      | 120.0 | BEA                         | 65.0 | MN                           | 6.0  | St                          | 29.0 |
| 8         | B1                      | 65.0 | SA                          | 67.0 | MN                           | 22.0 | St                          | 11.0 | 34        | B1                      | 100.0 | BEA                         | 65.0 | MN                           | 6.0  | St                          | 29.0 |
| 9         | B1                      | 65.0 | MYA                         | 67.0 | MN                           | 22.0 | St                          | 11.0 | 35        | B1                      | 50.0  | BEA                         | 65.0 | MN                           | 6.0  | St                          | 29.0 |
| 10        | B1                      | 65.0 | OA                          | 67.0 | MN                           | 22.0 | St                          | 11.0 | 36        | B1                      | 30.0  | BEA                         | 65.0 | MN                           | 6.0  | St                          | 29.0 |
| 11        | B1                      | 65.0 | BEA                         | 63.0 | MN                           | 7.0  | St                          | 23.0 | 37        | B1                      | 65.0  | BEA                         | 67.0 | MN                           | 22.0 | St                          | 11.0 |
|           |                         |      |                             |      | AA                           | 7.0  |                             |      | 38        | B1                      | 65.0  | BEA                         | 67.0 | MN                           | 22.0 | St                          | 11.0 |
| 12        | B1                      | 65.0 | BEA                         | 63.0 | MN                           | 15.0 | St                          | 15.0 | 39        | B1                      | 65.0  | BEA                         | 67.0 | MN                           | 22.0 | St                          | 11.0 |
|           |                         |      |                             |      | AA                           | 7.0  |                             |      | 40        | B1                      | 65.0  | BEA                         | 67.0 | MN                           | 22.0 | St                          | 11.0 |
| 13        | B1                      | 65.0 | BEA                         | 47.0 | MN                           | 22.0 | St                          | 11.0 | 41        | B1                      | 65.0  | BEA                         | 67.0 | MN                           | 22.0 | St                          | 11.0 |
|           |                         |      |                             | SA   | 20.0                         |      |                             | 42   | B1        | 65.0                    | BEA   | 67.0                        | MN   | 22.0                         | St   | 11.0                        |      |
| 14        | B1                      | 65.0 | BEA                         | 33.0 | MN                           | 22.0 | St                          | 11.0 | 43        | B1                      | 65.0  | BEA                         | 40.0 | AN                           | 27.5 | St                          | 30.0 |
|           |                         |      |                             | BEMA | 34.0                         |      |                             |      | 44        | B1                      | 65.0  | BEA                         | 40.0 | AN                           | 27.5 | St                          | 30.0 |
| 15        | B1                      | 65.0 | BEA                         | 17.0 | MN                           | 35.0 | St                          | 48.0 |           |                         |       |                             | UR   | 2.5                          |      |                             |      |
| 16        | B1                      | 65.0 | BEA                         | 30.0 | MN                           | 35.0 | St                          | 35.0 |           |                         |       |                             |      |                              |      |                             |      |
| 17        | B1                      | 65.0 | BEA                         | 52.0 | MN                           | 26.0 | St                          | 22.0 | 45        | B1                      | 65.0  | BEA                         | 67.0 | AA                           | 5.0  | MM                          | 29.0 |
| 18        | B1                      | 65.0 | BEA                         | 80.0 | MN                           | 15.0 | St                          | 5.0  | 46        | —                       | 0.0   | BEA                         | 67.0 | AA                           | 5.0  | MM                          | 29.0 |
| 19        | B1                      | 65.0 | BEA                         | 65.0 | MN                           | 15.0 | St                          | 20.0 | 47        | B9                      | 65.0  | BEA                         | 34.0 | MN                           | 11.0 | St                          | 55.0 |
| 20        | B1                      | 65.0 | BEA                         | 65.0 | MN                           | 6.0  | St                          | 29.0 | 48        | B11                     | 65.0  | BEA                         | 17.0 | MN                           | 35.0 | St                          | 48.0 |
| 21        | B1                      | 65.0 | BEA                         | 68.0 | MN                           | 32.0 | St                          | 0.0  | 49        | B1                      | 65.0  | HA                          | 61.0 | MN                           | 26.0 | St                          | 13.0 |
| 22        | B1                      | 65.0 | BEA                         | 88.0 | MN                           | 4.0  | St                          | 8.0  | 50        | B1                      | 65.0  | BEA                         | 60.0 | MM                           | 29.0 | —                           | —    |
| 23        | B1                      | 65.0 | BEA                         | 20.0 | MN                           | 80.0 | St                          | 0.0  |           |                         |       |                             | St   | 11.0                         |      |                             |      |
| 24        | B1                      | 65.0 | BEA                         | 17.0 | MN                           | 12.0 | St                          | 71.0 |           |                         |       |                             |      |                              |      |                             |      |
| 25        | B2                      | 65.0 | BEA                         | 65.0 | MN                           | 6.0  | St                          | 29.0 |           |                         |       |                             |      |                              |      |                             |      |
| 26        | B2                      | 65.0 | BEA                         | 65.0 | MN                           | 6.0  | St                          | 20.0 | 50        |                         |       |                             |      |                              |      |                             |      |

\* For toner 50 only, MM and St are handled as the second polymerizable monomer for the sake of convenience. The same applies for Table 3.

TABLE 3

| Polymer A |                        |                    |                   |                     |                   |                    |                   |                                    |                                    |                     |                   |
|-----------|------------------------|--------------------|-------------------|---------------------|-------------------|--------------------|-------------------|------------------------------------|------------------------------------|---------------------|-------------------|
| Toner No. | Inorganic particle No. | First monomer unit |                   | Second monomer unit |                   | Third monomer unit |                   | Weight-average                     |                                    |                     |                   |
|           |                        | Type               | Molar ratio mol % | Type                | Molar ratio mol % | Type               | Molar ratio mol % | SP <sub>21</sub> -SP <sub>11</sub> | SP <sub>22</sub> -SP <sub>12</sub> | molecular weight Mw | Melting point °C. |
| 1         | B1                     | BEA                | 28.88             | MN                  | 53.80             | St                 | 17.33             | 7.71                               | 4.28                               | 56000               | 62 100            |
| 2         | B1                     | BEA                | 25.28             | AN                  | 59.55             | St                 | 15.17             | 11.19                              | 5.05                               | 55500               | 62 100            |
| 3         | B1                     | BEA                | 26.02             | HPMA                | 54.96             | St                 | 19.02             | 5.87                               | 4.36                               | 53400               | 59 100            |
| 4         | B1                     | BEA                | 26.18             | VA                  | 57.87             | St                 | 15.95             | 3.35                               | 0.61                               | 53600               | 56 100            |
| 5         | B1                     | BEA                | 26.18             | MA                  | 57.87             | St                 | 15.95             | 3.35                               | 0.61                               | 54700               | 54 100            |

TABLE 3-continued

| Toner<br>No. | Inorganic<br>fine<br>particle<br>No. | Polymer A                |                         |                           |                         |                          |                         |                                    |                                    |                           |                          |
|--------------|--------------------------------------|--------------------------|-------------------------|---------------------------|-------------------------|--------------------------|-------------------------|------------------------------------|------------------------------------|---------------------------|--------------------------|
|              |                                      | First<br>monomer<br>unit |                         | Second<br>monomer<br>unit |                         | Third<br>monomer<br>unit |                         | Weight-<br>average                 |                                    |                           |                          |
|              |                                      | Type                     | Molar<br>ratio<br>mol % | Type                      | Molar<br>ratio<br>mol % | Type                     | Molar<br>ratio<br>mol % | SP <sub>21</sub> -SP <sub>11</sub> | SP <sub>22</sub> -SP <sub>12</sub> | molecular<br>weight<br>Mw | Melting<br>point<br>° C. |
| 6            | B1                                   | BEA                      | 27.61                   | AM                        | 56.87                   | St                       | 15.53                   | 21.01                              | 11.43                              | 56800                     | 59 100                   |
| 7            | B1                                   | BEA                      | 27.40                   | AA                        | 21.36                   | MM                       | 51.24                   | 10.47                              | 4.97                               | 57100                     | 57 100                   |
| 8            | B1                                   | SA                       | 32.26                   | MN                        | 51.24                   | St                       | 16.50                   | 7.57                               | 4.25                               | 55400                     | 54 100                   |
| 9            | B1                                   | MYA                      | 23.87                   | MN                        | 57.58                   | St                       | 18.55                   | 7.88                               | 4.32                               | 51800                     | 76 100                   |
| 10           | B1                                   | OA                       | 24.95                   | MN                        | 56.76                   | St                       | 18.28                   | 7.85                               | 4.32                               | 53400                     | 78 100                   |
| 11           | B1                                   | BEA                      | 28.16                   | MN                        | 17.75                   | St                       | 37.57                   | 7.71                               | 4.28                               | 55900                     | 58 100                   |
|              |                                      |                          |                         | AA                        | 16.52                   |                          |                         | 10.47                              | 4.97                               |                           |                          |
| 12           | B1                                   | BEA                      | 26.26                   | MN                        | 35.47                   | St                       | 22.85                   | 7.71                               | 4.28                               | 52900                     | 61 100                   |
|              |                                      |                          |                         | AA                        | 15.41                   |                          |                         | 10.47                              | 4.97                               |                           |                          |
| 13           | B1                                   | BEA                      | 19.96                   | MN                        | 53.01                   | St                       | 17.07                   | 7.67                               | 4.27                               | 53800                     | 58 100                   |
|              |                                      | SA                       | 9.96                    |                           |                         |                          |                         |                                    |                                    |                           |                          |
| 14           | B1                                   | BEA                      | 14.30                   | MN                        | 54.08                   | St                       | 17.42                   | 7.79                               | 4.32                               | 57400                     | 62 100                   |
|              |                                      | BEMA                     | 14.21                   |                           |                         |                          |                         |                                    |                                    |                           |                          |
| 15           | B1                                   | BEA                      | 4.35                    | MN                        | 50.78                   | St                       | 44.87                   | 7.71                               | 4.28                               | 52100                     | 54 100                   |
| 16           | B1                                   | BEA                      | 8.42                    | MN                        | 55.70                   | St                       | 35.88                   | 7.71                               | 4.28                               | 52800                     | 55 100                   |
| 17           | B1                                   | BEA                      | 18.58                   | MN                        | 52.70                   | St                       | 28.73                   | 7.71                               | 4.28                               | 55300                     | 59 100                   |
| 18           | B1                                   | BEA                      | 43.63                   | MN                        | 46.41                   | St                       | 9.97                    | 7.71                               | 4.28                               | 55800                     | 62 100                   |
| 19           | B1                                   | BEA                      | 29.12                   | MN                        | 38.13                   | St                       | 32.75                   | 7.71                               | 4.28                               | 55200                     | 62 100                   |
| 20           | B1                                   | BEA                      | 31.70                   | MN                        | 16.60                   | St                       | 51.70                   | 7.71                               | 4.28                               | 54200                     | 58 100                   |
| 21           | B1                                   | BEA                      | 27.25                   | MN                        | 72.75                   | St                       | 0.00                    | 7.71                               | 4.28                               | 57500                     | 62 100                   |
| 22           | B1                                   | BEA                      | 62.89                   | MN                        | 16.22                   | St                       | 20.90                   | 7.71                               | 4.28                               | 54400                     | 62 100                   |
| 23           | B1                                   | BEA                      | 4.22                    | MN                        | 95.78                   | St                       | 0.00                    | 7.71                               | 4.28                               | 54800                     | 55 100                   |
| 24           | B1                                   | BEA                      | 4.93                    | MN                        | 19.76                   | St                       | 75.31                   | 7.71                               | 4.28                               | 53800                     | 55 100                   |
| 25           | B2                                   | BEA                      | 31.70                   | MN                        | 16.60                   | St                       | 51.70                   | 7.71                               | 4.28                               | 53900                     | 58 100                   |
| 26           | B3                                   | BEA                      | 31.70                   | MN                        | 16.60                   | St                       | 51.70                   | 7.71                               | 4.28                               | 53900                     | 58 100                   |
| 27           | B4                                   | BEA                      | 31.70                   | MN                        | 16.60                   | St                       | 51.70                   | 7.71                               | 4.28                               | 53900                     | 58 100                   |
| 28           | B5                                   | BEA                      | 31.70                   | MN                        | 16.60                   | St                       | 51.70                   | 7.71                               | 4.28                               | 53900                     | 58 100                   |
| 29           | B6                                   | BEA                      | 31.70                   | MN                        | 16.60                   | St                       | 51.70                   | 7.71                               | 4.28                               | 53900                     | 58 100                   |
| 30           | B7                                   | BEA                      | 31.70                   | MN                        | 16.60                   | St                       | 51.70                   | 7.71                               | 4.28                               | 53900                     | 58 100                   |
| 31           | B8                                   | BEA                      | 31.70                   | MN                        | 16.60                   | St                       | 51.70                   | 7.71                               | 4.28                               | 53900                     | 58 100                   |
| 32           | B10                                  | BEA                      | 31.70                   | MN                        | 16.60                   | St                       | 51.70                   | 7.71                               | 4.28                               | 53900                     | 58 100                   |
| 33           | B1                                   | BEA                      | 31.70                   | MN                        | 16.60                   | St                       | 51.70                   | 7.71                               | 4.28                               | 53900                     | 58 100                   |
| 34           | B1                                   | BEA                      | 31.70                   | MN                        | 16.60                   | St                       | 51.70                   | 7.71                               | 4.28                               | 53900                     | 58 100                   |
| 35           | B1                                   | BEA                      | 31.70                   | MN                        | 16.60                   | St                       | 51.70                   | 7.71                               | 4.28                               | 53900                     | 58 100                   |
| 36           | B1                                   | BEA                      | 31.70                   | MN                        | 16.60                   | St                       | 51.70                   | 7.71                               | 4.28                               | 53900                     | 58 100                   |
| 37           | B1                                   | BEA                      | 28.88                   | MN                        | 53.80                   | St                       | 17.33                   | 7.71                               | 4.28                               | 68400                     | 62 100                   |
| 38           | B1                                   | BEA                      | 28.88                   | MN                        | 53.80                   | St                       | 17.33                   | 7.71                               | 4.28                               | 68400                     | 62 100                   |
| 39           | B1                                   | BEA                      | 28.88                   | MN                        | 53.80                   | St                       | 17.33                   | 7.71                               | 4.28                               | 68400                     | 62 100                   |
| 40           | B1                                   | BEA                      | 28.88                   | MN                        | 53.80                   | St                       | 17.33                   | 7.71                               | 4.28                               | 68400                     | 62 82                    |
| 41           | B1                                   | BEA                      | 28.88                   | MN                        | 53.80                   | St                       | 17.33                   | 7.71                               | 4.28                               | 68400                     | 62 52                    |
| 42           | B1                                   | BEA                      | 28.88                   | MN                        | 53.80                   | St                       | 17.33                   | 7.71                               | 4.28                               | 68400                     | 62 48                    |
| 43           | B1                                   | BEA                      | 11.36                   | AN                        | 56.05                   | St                       | 31.15                   | 11.19                              | 5.05                               | 53600                     | 55 100                   |
|              |                                      |                          |                         | UT                        | 1.44                    |                          |                         | 5.54                               | 4.21                               |                           |                          |
| 44           | B1                                   | BEA                      | 11.42                   | AN                        | 56.32                   | St                       | 31.30                   | 11.19                              | 5.05                               | 55400                     | 55 100                   |
|              |                                      |                          |                         | UR                        | 0.96                    |                          |                         | 3.50                               | 3.17                               |                           |                          |
| 45           | B1                                   | BEA                      | 32.90                   | AA                        | 12.97                   | MM                       | 54.13                   | 10.47                              | 4.97                               | 52700                     | 56 100                   |
| 46           |                                      | BEA                      | 32.90                   | AA                        | 12.97                   | MM                       | 54.13                   | 10.47                              | 4.97                               | 52700                     | 56 100                   |
| 47           | B9                                   | BEA                      | 11.43                   | MN                        | 20.98                   | St                       | 67.59                   | 7.71                               | 4.28                               | 56000                     | 62 100                   |
| 48           | B11                                  | BEA                      | 4.35                    | MN                        | 50.78                   | St                       | 44.87                   | 7.71                               | 4.28                               | 56000                     | 62 100                   |
| 49           | B1                                   | HA                       | 28.65                   | MN                        | 53.97                   | St                       | 17.38                   | 7.49                               | 4.24                               | 52200                     | 45 100                   |
| 50           | B1                                   | BEA                      | 28.51                   | MM                        | 52.39                   | —                        | —                       | 2.06                               | 0.58                               | 56500                     | 52 100                   |
|              |                                      |                          |                         | St                        | 19.1                    |                          |                         | 1.86                               | 0.25                               |                           |                          |

\*2: Percentage (mass %) of polymer a in the binder resin

TABLE 4

| First polymerizable<br>monomer |                      |  | SP value of<br>polymerizable<br>monomer<br>(J/cm <sup>3</sup> ) <sup>0.5</sup> | SP value of<br>monomer unit<br>(J/cm <sup>3</sup> ) <sup>0.5</sup> |
|--------------------------------|----------------------|--|--------------------------------------------------------------------------------|--------------------------------------------------------------------|
|                                |                      |  |                                                                                |                                                                    |
|                                | Behenyl acrylate     |  | 17.69                                                                          | 18.25                                                              |
|                                | Behenyl methacrylate |  | 17.61                                                                          | 18.10                                                              |
|                                | Stearyl acrylate     |  | 17.71                                                                          | 18.39                                                              |
|                                | Myricyl acrylate     |  | 17.65                                                                          | 18.08                                                              |
|                                | Octacosyl acrylate   |  | 17.65                                                                          | 18.10                                                              |
|                                | Hexadecyl acrylate   |  | 17.73                                                                          | 18.47                                                              |

TABLE 4-continued

|                                 |                                | SP value of<br>polymerizable<br>monomer<br>(J/cm <sup>3</sup> ) <sup>0.5</sup> | SP value of<br>monomer unit<br>(J/cm <sup>3</sup> ) <sup>0.5</sup> |
|---------------------------------|--------------------------------|--------------------------------------------------------------------------------|--------------------------------------------------------------------|
| Second polymerizable<br>monomer | Acrylonitrile                  | 22.75                                                                          | 29.43                                                              |
|                                 | Methacrylonitrile              | 21.97                                                                          | 25.96                                                              |
|                                 | Acrylic acid                   | 22.66                                                                          | 28.72                                                              |
|                                 | Methacrylic acid               | 21.95                                                                          | 25.65                                                              |
|                                 | 2-hydroxypropyl methacrylate   | 22.05                                                                          | 24.12                                                              |
|                                 | Vinyl acetate                  | 18.31                                                                          | 21.60                                                              |
|                                 | Methyl acrylate                | 18.31                                                                          | 21.60                                                              |
|                                 | Acrylamide                     | 29.13                                                                          | 39.25                                                              |
|                                 | Urethane group-bearing monomer | 21.91                                                                          | 23.79                                                              |
|                                 | Urea group-bearing monomer     | 20.86                                                                          | 21.74                                                              |
| Third polymerizable<br>monomer  | Styrene                        | 17.94                                                                          | 20.11                                                              |
|                                 | Methyl methacrylate            | 18.27                                                                          | 20.31                                                              |

TABLE 5

|            | Polymer<br>dispersion<br>Parts | Amorphous<br>resin<br>dispersion<br>Parts | Release<br>agent<br>dispersion<br>Parts | Inorganic<br>fine particle<br>dispersion<br>Parts |
|------------|--------------------------------|-------------------------------------------|-----------------------------------------|---------------------------------------------------|
| Example 32 | 500.0                          | —                                         | 50.0                                    | 650.0                                             |
| Example 40 | 410.0                          | 90.0                                      | 50.0                                    | 650.0                                             |

TABLE 5-continued

|            | Polymer<br>dispersion<br>Parts | Amorphous<br>resin<br>dispersion<br>Parts | Release<br>agent<br>dispersion<br>Parts | Inorganic<br>fine particle<br>dispersion<br>Parts |
|------------|--------------------------------|-------------------------------------------|-----------------------------------------|---------------------------------------------------|
| Example 41 | 260.0                          | 240.0                                     | 50.0                                    | 650.0                                             |
| Example 42 | 240.0                          | 260.0                                     | 50.0                                    | 650.0                                             |

TABLE 6

| Toner      | No. | Low-<br>temperature |      | Heat-<br>resistant<br>storability |      | Durability | Discharged<br>paper<br>adhesion |          | LL | HH |
|------------|-----|---------------------|------|-----------------------------------|------|------------|---------------------------------|----------|----|----|
|            |     | fixability          | Rank | Value                             | Rank |            | behavior                        | ghosting |    |    |
| Example 1  | 1   | A                   | A    | 15                                | A    | A          | A                               | A        | A  | A  |
| Example 2  | 2   | A                   | A    | 18                                | A    | A          | A                               | A        | A  | A  |
| Example 3  | 3   | A                   | B    | 22                                | A    | B          | A                               | A        | A  | A  |
| Example 4  | 4   | A                   | B    | 23                                | A    | C          | A                               | A        | A  | A  |
| Example 5  | 5   | A                   | C    | 28                                | A    | C          | A                               | A        | A  | A  |
| Example 6  | 6   | B                   | B    | 23                                | A    | A          | A                               | A        | A  | A  |
| Example 7  | 7   | A                   | C    | 28                                | C    | C          | A                               | A        | A  | A  |
| Example 8  | 8   | A                   | C    | 26                                | A    | A          | A                               | A        | A  | A  |
| Example 9  | 9   | C                   | A    | 18                                | A    | A          | A                               | A        | A  | A  |
| Example 10 | 10  | C                   | A    | 17                                | A    | A          | A                               | A        | A  | A  |
| Example 11 | 11  | A                   | B    | 23                                | A    | A          | A                               | A        | A  | A  |
| Example 12 | 12  | A                   | A    | 17                                | A    | A          | A                               | A        | A  | A  |
| Example 13 | 13  | A                   | B    | 24                                | A    | A          | A                               | A        | A  | A  |
| Example 14 | 14  | A                   | A    | 17                                | A    | A          | A                               | A        | A  | A  |
| Example 15 | 15  | C                   | C    | 27                                | A    | B          | A                               | A        | A  | A  |
| Example 16 | 16  | B                   | C    | 25                                | A    | B          | A                               | A        | A  | A  |
| Example 17 | 17  | B                   | B    | 22                                | A    | A          | A                               | A        | A  | A  |
| Example 18 | 18  | A                   | A    | 14                                | B    | A          | A                               | A        | A  | A  |
| Example 19 | 19  | A                   | A    | 17                                | B    | A          | A                               | A        | A  | A  |
| Example 20 | 20  | A                   | B    | 23                                | B    | A          | A                               | A        | A  | A  |
| Example 21 | 21  | B                   | A    | 15                                | A    | A          | A                               | A        | A  | A  |
| Example 22 | 22  | A                   | B    | 21                                | C    | A          | A                               | A        | A  | A  |
| Example 23 | 23  | C                   | C    | 25                                | A    | C          | A                               | A        | A  | A  |
| Example 24 | 24  | C                   | C    | 29                                | B    | C          | A                               | A        | A  | A  |
| Example 25 | 25  | A                   | B    | 23                                | C    | A          | A                               | A        | A  | A  |
| Example 26 | 26  | A                   | B    | 23                                | B    | B          | A                               | A        | A  | A  |
| Example 27 | 27  | A                   | C    | 29                                | B    | C          | A                               | A        | A  | A  |
| Example 28 | 28  | A                   | B    | 23                                | C    | C          | A                               | A        | A  | A  |
| Example 29 | 29  | A                   | B    | 22                                | B    | A          | B                               | A        | A  | A  |
| Example 30 | 30  | A                   | B    | 23                                | B    | B          | A                               | A        | C  | A  |
| Example 31 | 31  | A                   | B    | 22                                | B    | C          | A                               | A        | C  | A  |
| Example 32 | 32  | A                   | B    | 21                                | B    | B          | B                               | C        | A  | A  |
| Example 33 | 33  | C                   | A    | 13                                | A    | A          | A                               | A        | A  | A  |
| Example 34 | 34  | B                   | A    | 14                                | A    | A          | A                               | A        | A  | A  |
| Example 35 | 35  | A                   | A    | 18                                | B    | A          | A                               | A        | A  | A  |
| Example 36 | 36  | A                   | A    | 19                                | C    | B          | A                               | A        | B  | A  |
| Example 37 | 37  | A                   | A    | 18                                | A    | A          | A                               | A        | A  | A  |
| Example 38 | 38  | A                   | A    | 19                                | A    | A          | A                               | A        | A  | A  |
| Example 39 | 39  | A                   | A    | 18                                | A    | A          | A                               | A        | A  | A  |

TABLE 6-continued

| Toner                 | Low-temperature |            | Heat-resistant storability |       | Durability | Discharged paper adhesion |          |          |
|-----------------------|-----------------|------------|----------------------------|-------|------------|---------------------------|----------|----------|
|                       | No.             | fixability | Rank                       | Value |            | Rank                      | behavior | ghosting |
| Example 40            | 40              | A          | A                          | 17    | A          | A                         | A        | A        |
| Example 41            | 41              | B          | A                          | 17    | A          | A                         | A        | A        |
| Example 42            | 42              | C          | A                          | 18    | A          | A                         | A        | A        |
| Example 43            | 43              | C          | C                          | 27    | A          | B                         | A        | A        |
| Example 44            | 44              | C          | C                          | 27    | A          | B                         | A        | A        |
| Example 45            | 45              | A          | C                          | 28    | C          | C                         | A        | A        |
| Comparative Example 1 | 46              | A          | C                          | 29    | D          | D                         | A        | A        |
| Comparative Example 2 | 47              | C          | C                          | 29    | A          | D                         | A        | C        |
| Comparative Example 3 | 48              | D          | D                          | 31    | A          | C                         | A        | C        |
| Comparative Example 4 | 49              | A          | D                          | 30    | A          | A                         | A        | A        |
| Comparative Example 5 | 50              | A          | D                          | 31    | A          | D                         | A        | A        |

While the present invention has been described with reference to exemplary embodiments, it is to be understood that the invention is not limited to the disclosed exemplary embodiments. The scope of the following claims is to be accorded the broadest interpretation so as to encompass all such modifications and equivalent structures and functions.

This application claims the benefit of Japanese Patent Application No. 2019-099365, filed May 28, 2019 which is hereby incorporated by reference herein in its entirety.

What is claimed is:

1. A toner, comprising:

a toner particle that contains a binder resin and inorganic fine particles;  
the binder resin contains a polymer A that includes a first monomer unit derived from a first polymerizable monomer selected from the group consisting of (meth)acrylate esters having an alkyl group having 18 to 36 carbons, and a second monomer unit derived from a second polymerizable monomer that is different from the first polymerizable monomer;  
each of the inorganic fine particles contains a substrate containing at least one inorganic element selected from metal elements and metalloid elements, and a coating layer, wherein

$$3.00 \leq (SP_{21} - SP_{11}) \leq 25.00$$

where  $SP_{11}$  ( $J/cm^3$ )<sup>0.5</sup> is an SP value of the first monomer unit and  $SP_{21}$  ( $J/cm^3$ )<sup>0.5</sup> is an SP value of the second monomer unit, and  
the coating layer has a structure represented by at least one of the group consisting of formulae (A), (B), (C) and (D)



-continued

(C)



(D)

where M independently represents one or more elements selected from the group consisting of tetravalent Si, tetravalent Ti and tetravalent Zr, M' independently represents one or more elements selected from the group consisting of trivalent Ti, trivalent Zr and trivalent Al, R<sup>1</sup> independently represents an alkyl group or a derivative thereof, R<sup>2</sup> to R<sup>7</sup> independently represent a hydrogen atom, hydroxy group, —O—\* or a group selected from the group consisting of alkoxy groups, alkyl groups and derivatives thereof, \* represents a bonding segment to the inorganic element, and n and m independently represent a positive integer equal to or greater than 1.

2. The toner according to claim 1, wherein each of the inorganic fine particles is a reaction product of the substrate and a compound represented by formula (3)



(3)

where R' represents an alkoxy group, m represents an integer of 1 to 3, Y' represents an alkyl group or a derivative thereof, and n represents an integer of 1 to 3, with the proviso that m+n=4.

3. The toner according to claim 2, wherein, R' represents an alkoxy group and Y' represents an alkyl group having 1 to 20 carbons.

4. The toner according to claim 1, wherein a content of the first monomer unit in the polymer A is 5.00 mol % to 60.00 mol % with reference to a total number of moles of all monomer units in the polymer A, and  
a content of the second monomer unit in the polymer A is 20.00 mol % to 95.00 mol % with reference to the total number of moles of all monomer units in the polymer A.

## 51

5. The toner according to claim 1, wherein the second polymerizable monomer is at least one member selected from the group consisting of formulae (E) and (F)



where X represents a single bond or an alkylene group having 1 to 6 carbons,

R<sup>8</sup> represents —C≡N, —C(=O)NHR<sup>11</sup> where R<sup>11</sup> is a hydrogen atom or an alkyl group having 1 to 4 carbons, hydroxy group, —COOR<sup>12</sup> where R<sup>12</sup> is an alkyl group having 1 to 6 carbons or a hydroxylalkyl group having 1 to 6 carbons, —NHCOOR<sup>13</sup> where R<sup>13</sup> is an alkyl group having 1 to 4 carbons, —NH—C(=O)—N(R<sup>14</sup>)<sub>2</sub> where R<sup>14</sup> is independently a hydrogen atom or an alkyl group having 1 to 6 carbons, —COO(CH<sub>2</sub>)<sub>2</sub>NHCOOR<sup>15</sup> where R<sup>15</sup> is an alkyl group having 1 to 4 carbons, or —COO(CH<sub>2</sub>)<sub>2</sub>—NH—C(=O)—N(R<sup>16</sup>)<sub>2</sub> where R<sup>16</sup> is independently a hydrogen atom or an alkyl group having 1 to 6 carbons,

R<sup>9</sup> represents an alkyl group having 1 to 4 carbons, and R<sup>10</sup> represents a hydrogen atom or a methyl group.

6. The toner according to claim 1, wherein the second polymerizable monomer is at least one member selected from the group consisting of formulae (E) and (F)



where X represents a single bond or an alkylene group having 1 to 6 carbons,

R<sup>8</sup> represents a nitrile group —C≡N, —C(=O)NHR<sup>11</sup> where R<sup>11</sup> is a hydrogen atom or an alkyl group having 1 to 4 carbons, hydroxy group, —COOR<sup>12</sup> where R<sup>12</sup> is an alkyl group having 1 to 6 carbons or a hydroxylalkyl group having 1 to 6 carbons, —NH—C(=O)—N(R<sup>14</sup>)<sub>2</sub> where R<sup>14</sup> is independently a hydrogen atom or an alkyl group having 1 to 6 carbons, —COO

(CH<sub>2</sub>)<sub>2</sub>NHCOOR<sup>15</sup> where R<sup>15</sup> is an alkyl group having 1 to 4 carbons, or —COO(CH<sub>2</sub>)<sub>2</sub>—NH—C(=O)—N(R<sup>16</sup>)<sub>2</sub> where R<sup>16</sup> is independently a hydrogen atom or an alkyl group having 1 to 6 carbons

5 R<sup>9</sup> represents an alkyl group having 1 to 4 carbons, and R<sup>10</sup> represents a hydrogen atom or a methyl group.

7. The toner according to claim 1, wherein the polymer A includes a third monomer unit derived from a third polymerizable monomer that is different from both the first and second polymerizable monomers, and

the third polymerizable monomer is at least one member selected from the group consisting of styrene, methyl methacrylate and methyl acrylate.

15 8. The toner according to claim 1, wherein the substrate is a metal oxide or a metalloid oxide.

9. The toner according to claim 1, wherein the substrate is magnetite.

20 10. The toner according to claim 1, wherein

$$1.5 \leq Z \leq 10.0 \text{ and } Y-X \geq 0.10$$

where X is an amount of moisture adsorption (mg/g) for an adsorption curve of the inorganic fine particles at 30.0° C. and 10% relative humidity,

Y is an amount of moisture adsorption (mg/g) for a desorption curve of the inorganic fine particles at 30.0° C. and 10% relative humidity, and

Z is an amount of moisture adsorption (mg/g) of the inorganic fine particles at 30.0° C. and 100% relative humidity.

35 11. The toner according to claim 1, wherein the inorganic fine particles contain 0.30 to 2.50 mass % carbon.

12. The toner according to claim 1, wherein the toner particle is a suspension-polymerized toner particle.

40 13. A method of producing the toner according to claim 1, comprising the steps of:

forming in an aqueous medium a particle of a polymerizable monomer composition that contains a polymerizable monomer; and

polymerizing the polymerizable monomer contained in the particle to obtain the toner particle containing polymer A obtained.

45 14. A toner, comprising:

a toner particle that contains a binder resin and inorganic fine particles

the binder resin contains a polymer A that is a polymer of a composition containing a first polymerizable monomer selected from the group consisting of (meth) acrylate esters having an alkyl group having 18 to 36 carbons, and a second polymerizable monomer that is different from the first polymerizable monomer;

50 55 each of the inorganic fine particles contains a substrate containing at least one inorganic element selected from metal elements and metalloid elements, and a coating layer, wherein

$$0.60 \leq (SP_{22} - SP_{12}) \leq 15.00$$

60 where SP<sub>12</sub> (J/cm<sup>3</sup>)<sup>0.5</sup> is an SP value of the first polymerizable monomer and SP<sub>22</sub> (J/cm<sup>3</sup>)<sup>0.5</sup> is an SP value of the second polymerizable monomer, and

the coating layer has a structure represented by at least one of the group consisting of formulae (A), (B), (C) and (D)



where M independently represents one or more elements selected from the group consisting of tetravalent Si, tetravalent Ti and tetravalent Zr, M' independently represents one or more elements selected from the group consisting of trivalent Ti, trivalent Zr and trivalent Al, R<sup>1</sup> independently represents an alkyl group or a derivative thereof, R<sup>2</sup> to R<sup>7</sup> independently represent a hydrogen atom, hydroxy group, —O—\* or a group selected from the group consisting of alkoxy groups, alkyl groups and derivatives thereof; \* represents a

bonding segment to the inorganic element, and n and m independently represent a positive integer equal to or greater than 1.

15. The toner according to claim 14, wherein a content of the first polymerizable monomer in the composition is 5.00 to 60.00 mol % with reference to a total number of moles for all the polymerizable monomer in the composition, and a content of the second polymerizable monomer in the composition is 20.00 to 95.00 mol % with reference to the total number of moles for all the polymerizable monomer in the composition.

16. A toner, comprising:  
 a toner particle that contains a binder resin and inorganic fine particles;  
 the binder resin contains a polymer A that includes a first monomer unit derived from a first polymerizable monomer selected from the group consisting of (meth) acrylate esters having an alkyl group having 18 to 36 carbons, and a second monomer unit derived from a second polymerizable monomer that is different from the first polymerizable monomer; and  
 each of the inorganic fine particles contains a substrate containing at least one inorganic element selected from metal elements and metalloid elements, wherein

$$3.00 \leq (SP_{21} - SP_{11}) \leq 25.00$$

where  $SP_{11}$  (J/cm<sup>3</sup>)<sup>0.5</sup> is designates an SP value of the first monomer unit and  $SP_{21}$  (J/cm<sup>3</sup>)<sup>0.5</sup> is an SP value of the second monomer unit, and  
 the substrate has been treated with a compound that has an alkoxy group and an alkyl group.

17. The toner according to claim 16, wherein the substrate has been treated with a compound represented by formula (3)

$$R'mSiY'n$$

(3)

where R' represents an alkoxy group, m represents an integer of 1 to 3, Y' represents an alkyl group or a derivative thereof, and n represents an integer of 1 to 3; with the proviso that m+n=4.

\* \* \* \* \*